# EUROPEAN PATENT SPECIFICATION

(11) **EP 1 522 900 B1**
(45) Date of publication and mention of the grant of the patent: **06.08.2008**
(21) Application number: 04256240.5
(22) Date of filing: 08.10.2004
(51) Int. Cl.: G03G 9/08

(54) **Toner and developer, and image forming method and apparatus using the developer**
Toner und Entwickler, sowie ein Bildherstellungsverfahren und Apparat, worin der Entwickler eingesetzt wird
Toner et révélateur,ainsi que procédé et appareil de production d' images utilisant ledit révélateur

(30) Priority: 08.10.2003 JP 2003349060; 28.11.2003 JP 2003400263
(43) Date of publication of application: 13.04.2005
(73) Proprietor: Ricoh Company, Ltd., Tokyo 143-8555 (JP)
(72) Inventor: Yamada, Hiroshi, Numazu-shi Shizuoka-ken (JP); Tomita, Masami, Numazu-shi Shizuoka-ken (JP); Nanya, Toshiki, Mishima-shi Shizuoka-ken (JP); Sasaki, Fumihiro, Fuji-shi Shizuoka-ken (JP); Emoto, Shigeru, Numazu-shi Shizuoka-ken (JP); Shimota, Naohito, Suntou-gun Shizuoka-ken (JP); Yagi, Shinichiro, Numazu-shi Shizuoka-ken (JP); Higuchi, Hiroto, Numazu-shi Shizuoka-ken (JP); Suzuki, Tomomi, Numazu-shi Shizuoka-ken (JP); Awamura, Junichi, Shizuoka-ken (JP); Honda, Takahiro, Numazu-shi Shizuoka-ken (JP)
(74) Representative: Lamb, Martin John Carstairs

(56) References cited:
- EP-A- 0 590 314
- EP-A- 0 943 658
- EP-A- 1 026 554
- EP-A- 1 273 977
- EP-A- 1 296 201
- EP-A- 1 308 791
- US-A- 5 017 450

## Description

### BACKGROUND OF THE INVENTION

### Field of the Invention

The present invention relates to a toner for use in a developer for developing an electrostatic latent image in electrophotography, electrostatic recording and electrostatic printing and the like, and to an electrophotographic image forming method and an image forming apparatus using the toner.

### Discussion of the Background

A developer for use in the electrostatic latent image in electrophotography, electrostatic recording and electrostatic printing and the like is adhered to an image bearer such as a photoreceptor on which an electrostatic latent image is formed in a development process; transferred therefrom onto a transfer medium such as a transfer paper in a transfer process; and fixed on the transfer medium in a fixing process. The developer for developing the electrostatic latent image formed on the image bearer includes a two-component developer formed of a carrier and a toner; and a one-component developer without a carrier, i.e., a magnetic or a non-magnetic toner.

Conventionally, a dry toner for use therein is formed by kneading a toner binder such as a styrene resin and a polyester resin with a colorant upon application of heat to form a kneaded mixture, cooling the mixture to solidify the mixture and pulverizing the solidified mixture.

A particle diameter of the toner is downsized to produce high-definition and high-quality images. However, a toner formed by the conventional kneading and pulverizing method has an amorphous particle form and cannot be classified because ultrafine particles having a strong adherence keep adhering to a toner having a desired particle diameter even after a classifying process. In an image forming apparatus, such ultrafine particles adhere to a carrier and apparatus parts and are fixed thereon due to being stirred with the carrier in an image developer, and due to a contact stress to a developing roller, a toner feeding roller, a layer-thickness regulation blade and a frictional-charged blade; and in the meantime, a fluidizer is buried in the surface of the toner, resulting in quality deterioration of the resultant images. In addition, the amorphous toner having a low fluidity as a powder needs a large amount of the fluidizer and a filling rate thereof into a toner bottle is so low that the amorphous toner is one of impediments to downsizing of the apparatus. Therefore, the toner having a small particle diameter is not yet fully utilized. Further, the kneading and pulverizing method has a limit of the particle diameter, and is unable to further downsize the particle diameter.

Further, to stabilize various properties of the toner such as a chargeability thereof, a method of sharpening a distribution of the particle diameter thereof is used. However, the method does not work well when an average particle diameter of the toner and a specific particle diameter distribution do not match each other. Namely, the average particle diameter thereof is an average after all, and does not show a content of the toner having too small or large a particle diameter. In addition, a generalized and specified relationship therebetween is insufficient and the toner preferably has a specific particle diameter distribution and a shape in accordance with the average particle diameter, and further has a pertinent correlation with an external additive.

Further, to produce full-color images, a transfer process transferring an image formed of multiple color toners from a photoreceptor to a transfer medium and a paper is becoming complicated, and a large amount of the amorphous pulverized toner is consumed to catch up with an image omission because of its poor transferability.

However, a spheric toner cannot be removed with a cleaner removing a residual toner from the photoreceptor and transfer medium such as a cleaning blade and a cleaning brush and causes defective cleaning. In addition, the whole surface of the spheric toner is exposed outside and the spheric toner easily contacts the carrier and a charged member such as a charged blade. Therefore, an external additive and a charge controlling agent present on the surface of the toner are easily buried therein, resulting in deterioration of the fluidity of the toner.

Accordingly, demands for reducing a running cost and producing high-definition images without an image omission by improving transferability of the toner to decrease the consumption thereof are increasing. This is because better transferability of the toner can dispense with a cleaning unit to remove an untransferred toner from a photoreceptor and a transfer medium, and therefore the apparatus can be downsized, a cost thereof can be reduced and there is no waste toner at the same time. To remedy such disadvantages due to the shapes, methods of producing toners having various shapes are invented. A method of producing a toner by suspension polymerization only can produce a spheric or almost a spheric toner, and an ultrafine powder tends to be produced because an irregular shearing stress is applied to toner materials in a suspension dispersion in water, and therefore the resultant toner still has poor cleanability and adheres to the carrier and parts of apparatus. On the other hand, a method of producing a toner by emulsion polymerization can produce both an amorphous and a spheric toner. However, a shape of the toner after the polymerization needs to be controlled upon application of heat, and an ultrafine powder which has not agglutinated inwater tends to remain, and therefore the resultant toner still has poor cleanability and adheres to the carrier and parts of the apparatus. Further, each of the toners produced by these methods is not previously designed in consideration of its suitability to an external additive.

Japanese Laid-Open Patent Publication No. 7-152202 discloses a polymer dissolution suspension method accompanied with a volume contraction.

The method includes dispersing or dissolving toner materials in a volatile solvent such as a low-boiling organic solvent to form a dispersion or a solution; emulsifying the dispersion or solution in a water medium including a dispersant to be a droplet; and removing the volatile solvent therefrom. Then, a volume of the droplet contracts, and only amorphous particles are formed when a solid particulate dispersant which is not dissolved in the water medium is used as the dispersant.

When a solid content is increased to improve productivity, a viscosity of a dispersed phase increases, and the resultant particles have a large particle diameter and a broad distribution thereof. When the viscosity thereof is decreased by using a low-molecular-weight resin, fixability, particularly hot offset resistance of the resultant toner deteriorates.

Japanese Laid-Open Patent Publication No. 11-149179 discloses a method of decreasing the viscosity of the dispersed phase using a low-molecular-weight resin in the polymer dissolution suspension method to make the emulsification easier, and performing an inter-particle polymerization to improve the fixability of the resultant toner. However, this does not improve the transferability and cleanability thereof controlling the shape thereof.

In addition, an ultrafine powder tends to be produced because an irregular shearing stress is applied to toner materials in a suspension dispersion in water, and therefore the resultant toner still has poor cleanability and adheres to the carrier and parts of apparatus.

Toner compositions which include modified polyester and which have a specified shape are disclosed in EP-A-1308791, EP1026554, EP1273977 and EP0943658. Generally, these are spherical toners, though the toner particles disclosed in EP1308791 are described as spindle shaped.

A colour toner having a vinyl-modified polyester as binder resin is disclosed in US5017450. EP-A-0509314 discloses a low melt, low gloss toner resin comprising uncrosslinked portions and crosslinked portions, in which crosslinked portions consist essentially of high density crosslinked microgel particles, wherein the microgel particles are present in amount from about 20 to 45% by weight of the toner resin.

An image forming method and a toner composition for use in the method in which volume change and area change of a toner image in the fixer are controlled are disclosed in EP-A-1296201.

These dry toners are fixed on a transfer medium such as a paper upon application of heat with a heating roller after being transferred thereto. When the heating roller has too high a temperature, the toner is excessively melted and fusion-bonded thereon (hot offset). When the temperature is too low, the toner is not fully melted and not sufficiently fixed thereon.

In terms of saving energy and downsizing the apparatus, a toner having both a hot offset resistance and a low-temperature fixability is required. Further, the toner is required to have a thermostable preservability so as not to be blocked at an atmospheric temperature in the apparatus. Particularly, a toner for use in full-color copiers and printers is required to provide glossiness and color mixability, and therefore the toner needs to have a lower melting viscosity and a sharp melting polyester toner binder is used therein. However, such a toner has poor hot offset resistance, and therefore a silicone oil is typically applied to the heating roller of the full-color apparatus.

However, the method of applying the silicone oil to the heating roller needs an.oil tank and an oil applicator, which complicate and enlarge the apparatus. In addition, the heating roller deteriorates and needs a periodical maintenance. Further, the oil inevitably adheres to copy papers and OHP films, and particularly the oil impairs color tone of the OHP films.

Because of these reasons, a need exists for a. toner having a small particle diameter and good fluidity, developability and transferability, and producing high-quality images without filming for long periods, and having a long life.

### SUMMARY OF THE INVENTION

Accordingly, an object of the present invention is to provide a toner having a small particle diameter and good fluidity, developability and transferability, and producing high-quality images without filming for long periods, and having a long life.

Another object of the present invention is to provide a toner container filled with the toner, a developer including the toner, an image forming method and an image forming apparatus using the developer.

Briefly these objects and other objects of the present invention as hereinafter will become more readily apparent can be attained by a toner including a particulate toner material having an average circularity of from 0.93 to 0.99, and including amodifiedpolyesterbinderresin, andacolorant; andanexternal additive having a primary particle diameter of from 5 to 20 nm and a secondary particle diameter of from 50 to 200 nm, wherein the toner has a melting viscosity of from 70 to 140 Pa·s at 160 °C, a weight-average particle diameter (D4) of from 3 to 7 µm, a ratio (D4/Dn) of the weight-average particle diameter to a number-average particle diameter (Dn) of the toner of from 1.01 to 1.25, particles having a particle diameter not greater than 4 µm being present in an amount less than 10 % by number or particles having a particle diameter not less than 8 µm being present in an amount less than 2 % by volume, and wherein the toner includes the external additive in an amount of from 0.3 to 5.0 parts by weight per 100 parts by weight of the particulate toner material.

These and other objects, features and advantages of the present invention will become apparent upon consideration of the following description of the preferred embodiments of the present invention taken in conjunction with the accompanying drawings.

### BRIEF DESCRIPTION OF THE DRAWINGS

Various other objects, features and attendant advantages of the present invention will be more fully appreciated as the same becomes better understood from the detailed description when considered in connection with the accompanying drawings in which like reference characters designate like corresponding parts throughout and wherein:
Figs. 1A to 1D are schematic views illustrating embodiments of photosensitive layer compositions of the amorphous silicon photoreceptor for use in the present invention respectively;
Fig. 2 is a schematic view illustrating an embodiment of the image forming apparatus of the present invention;
Fig. 3 is a schematic view illustrating another embodiment of an image forming apparatus of the present invention;
Fig. 4 is a schematic view illustrating an embodiment of the process cartridge of the present invention;
Fig. 5 is a schematic view illustrating a third embodiment of the image forming apparatus using a surf fixer of the present invention;
Fig. 6 is a schematic view partially illustrating a fourth embodiment of the image forming apparatus using a charging roller as the contact charger of the present invention; and
Fig. 7 is a schematic view partially illustrating fifth embodiment of the image forming apparatus using a fur or a magnetic brush as the contact charger of the present invention.

### DETAILED DESCRIPTION OF THE INVENTION

Generally, the present invention provides a toner having a small particle diameter and good fluidity, developability and transferability, and producing high-quality images without filming for long periods, and having a long life.

Typically, when a modified polyester is produced in a process of dissolving or dispersing toner compositions including a prepolymer in an organic solvent to prepare a solution or a dispersion; and dispersing the solution or dispersion to form a toner, the toner has a core shell structure. The toner is kneaded upon application of heat with a shearing force between a heating roller and a back-up roller in a fixer. Therefore, a resin forming the core and having a low softening point is exposed outside and the melted toner contaminates an inside of the fixer, resulting in contamination of a transfer paper. The toner according to the invention has a melting viscosity of from 70 to 140 Pa·s at 160 °C. When less than 70 Pa·s, the melted toner contaminates an inside of the fixer, resulting in contamination of a transfer paper. When greater than 140 Pa · s, a cold offset problem occurs. It is difficult to solve these problems simply by controlling a thermal property of the toner, and it is necessary to repeat a melted and kneaded status of the toner in a fixer.

Typically, it is said that the smaller the toner particle diameter, the more advantageous to produce high-resolution and high-quality images. However, the more disadvantageous for transferability and cleanability of the toner, and which produce images having insufficient image density and stripes due to the poor cleanability. A toner having a weight-average particle diameter smaller than the range of the present invention is fusion bonded with the surface of a carrier in a two-component developer stirred for long periods in an image developer and the chargeability of the carrier deteriorates. When used in a one-component developer, a toner film over a charging roller tends to be formed and the toner tends to be fusion bonded with a member such as a blade forming a thin toner layer. Particularly, a quantitative balance of an ultrafine powder is lost, the toner tends to be more fusion bonded with the surface of a carrier, the toner film over a charging roller tends to be more formed and the toner tends to be more fusion bonded with a member such as a blade forming a thin toner layer. A toner including a modified polyester resin prevents these phenomena from occurring.

A toner having a particle diameter larger than the range of the present invention makes it difficult to produce high-resolution and high-quality images, and at the same time, a variation of particle diameter thereof becomes large in many cases when the toner is consumed and fed in a developer. This is the same when a ratio (D4/Dn) of the weight-average particle diameter (D4) to a number-average particle diameter of the toner is too high.

These problems are difficult to solve only by forming a toner having a sharp particle diameter distribution, a specific content of a fine powder and/or a specific content range of a coarse powder, and further the following specific shape range of a toner is indispensable.

Typically, when the toner has a shape close to a sphere, transferability thereof improves, but cleanability of the toner remaining on a photoreceptor after being transferred becomes worse. In the present invention, the toner preferably has an average sphericityof from 0.93 to 0.99 in addition to the particle diameter. When less than 0.93, the toner has a lowdevelopability and produces images having low image density. When larger than 0.99, the toner initially has a high developability and produces images having high image density, but the developability deteriorates when used for long periods and the image density largely deteriorates. When the spheric toner has the particle diameter of the present invention, an external additive and a charge controlling agent present on the surface thereof are difficult to bury therein. This is because it is supposed that a stress mechanically applied to a toner is dispersed and the stress on each particle of the toner extremely decreases even when the toner has a shape close to a sphere, provided the toner has a particle diameter distribution in a range of the present invention and a uniform particle diameter, since a toner having a large particle diameter tends to cause a phenomenon wherein an external additive and a charge controlling agent present on the surface of the toner bury therein. Particle diameter distributions are preferably measured using a Coulter counter, for example, a Coulter counter TA-II using an aperture of 100 micrometres to determine volume and number distribution. The weight average particle diameter D4 is suitably calculated based on the volume distribution.

The circularity of a toner particle is preferably calculated by determining the peripheral length of a circle having an area equivalent of that of a projected image optically detected and dividing the peripheral length of the circle by the actual peripheral length of the toner particle. For example, a flow-type particle image analyzer may be used. The average circularity is preferably a number average.

Similarly, the toner preferably has a shape factor (SF-1) of from 105 to 170. When greater than 170, the toner may be atomized after being stirred in an image developer for long periods, and therefore developability thereof may deteriorate and the toner produces foggy images, and further transferability thereof may deteriorate and the toner may produce images having low image density. When less than 105, the fluidity and chargeability of the toner changes because an external additive such as silica coated on the surface of the toner for the purpose of improving the fluidity thereof may be buried therein, and therefore developability thereof may deteriorate and the toner may produce foggy images, and further cleanability of the toner remaining on a photoreceptor after being transferred may become worse.

The shape factor (SF-1) of the toner represents a degree of roundness thereof, and is determined as follows: $SF - 1 = ( MXLNG ⁢ {)}^{2} / AREA \times π / 4 \times 100$
wherein MXLNG represents an absolute maximum length of a particle and AREA represents a projected area thereof.

The toner of the present invention includes an external additive having a primary particle diameter of from 5 to 20 nm and a secondary particle diameter of from 50 to 200 nm in an amount of from 0.3 to 5.0 parts by weight per 100 parts by weight of the mother toner. When less than 0.3 parts by weight, fluidity
of the resultant toner is insufficient and transferability thereof deteriorates. When greater than 5.0 parts by weight, the external additive is not fully adhered to the surface of the toner and some thereof is present. Therefore, the external additive alone adheres to and abrades the surface of a photoreceptor, which produces images having white spots and background fouling, and fixability of the resultant toner deteriorates.

The external additive having a primary particle diameter of from 5 to 20 nm and a secondary particle diameter of from 50 to 200 nm is preferably used to improve fluidity and chargeability of the resultant toner. The reason is not clarified, yet it is supposed that when the toner is fed in an image developer, the toner is present in a condensed state having a particle diameter of from 50 to 200 nm and is stably fed therein, and when stirred with a carrier in the image developer, the toner is disassembled and comes to a state of the primary particle which has a suitable developability when developing. In addition, an energy generated when being stirred with a carrier in the image developer is used to disassemble an aggregation of the external additive and changes of the various properties of the toner such as deterioration of the fluidity thereof can be prevented. Such an external additive includes inorganic particulate materials and particulate polymer materials.

Specific examples of the inorganic particles include silica, titanium dioxide, alumina, barium titanate, magnesium titanate, calcium titanate, strontium titanate, zinc oxide, tin oxide, quartz sand, clay, mica, sand-lime, diatomearth, chromium oxide, ceriumoxide, redironoxide, antimonytrioxide, magnesium oxide, zirconium oxide, barium sulfate, barium carbonate, calcium carbonate, silicon carbide, silicon nitride, etc.

Specific examples of the polymer particulate material include polystyrene formed by a soap-free emulsifying polymerization; a suspension polymerization or a dispersing polymerization, estermethacrylate or esteracrylate copolymers, silicone resins, benzoguanamine resins, polycondensation particles such as nylon and polymer particles of thermosetting resins.

A surface treatment agent can increase hydrophobicity of these fluidizers and prevent deterioration of fluidity and chargeability of the resultant toner even in high humidity. Specific examples of the surface treatment agent include silane coupling agents, sililating agents, silane coupling agents having an alkyl fluoride group, organic titanate coupling agents, aluminium coupling agents silicone oils and modified silicone oils.

Silica, titanium dioxide and alumina are preferably used, and particularly hydrophobized silica is more preferably used as the external additive in the present invention.

The modified polyester resin in the present invention includes a polyester resin wherein a group bonded with a functional group included in a monomer unit of an acid or alcohol in other manners than an ester bond is present; and a polyester resin wherein plural resin components having a different structure are bonded with each other in a covalent or an electrovalent bond, etc.

For example, a polyester resin having a functional group such as an isocyanate group (for reacting with an acid radical or a hydroxyl group) at an end thereof wherein the end is further modified or elongated with a compound including an active hydrogen atom is also used. Further, a polyester resin having ends bonded with a compound including plural hydrogen atoms such as a urea-modified polyester resin and a urethane-modified polyester resin may also be used.

In addition, a polyester resin having a reactive group such as double bonds in a main chain thereof, which is radically polymerized to have a graft component, i.e., a carbon to carbon combination or in which the double bonds are crosslinked with each other such as a styrene-modified polyester resin and an acrylic-modified polyester resins may also be used.

A polyester resin may be used which is copolymerised with a resin having a different composition, being copolymerized in a main chain thereof or reacted with a carboxyl group and a hydroxyl group at an end thereof, e.g., a polyester resin copolymerized with a silicone resin having an end modified by a carboxyl group, a hydroxyl group, an epoxy group and a mercapto group such as a silicone-modified polyester resin.

Hereinafter, the modified polyester resin will be more specifically explained.

### Synthesis example of a polystyrene-modified polyester resin

724 parts of an adduct of bisphenol A with 2 moles of ethyleneoxide, 200 parts isophthalic acid, 70 parts of fumaric acid and 2 parts of dibutyltinoxide are mixed and reacted in a reactor vessel including a cooling pipe, a stirrer and a nitrogen inlet pipe for 8 hrs at a normal pressure and 230 °C. Further, after the mixture is depressurized by 10 to 15 mm Hg and reacted for 5 hrs, 32 parts of phthalic acid anhydride are added thereto and reacted for 2 hrs at 160 °C. Next, 200 parts of styrene, 1 part of benzoyl peroxide, 0.5 parts of dimethylaniline dissolved in ethyl acetate are reacted with the mixture for 2 hrs at 80 °C, and the ethyl acetate is distilled and removed to prepare a polystyrene-graft-modified polyester resin (i) having a weight-average molecular weight of 92,000.

### Urea-modified polyester resin (i)

Specific examples of the urea-modified polyester resin (i) include reaction products between polyester prepolymers (A) having an isocyanate group and amines (B). The polyester prepolymer (A) is formed from a reaction between polyester having an active hydrogen atom formed by polycondensation between polyol (1) and a polycarboxylic acid (2), and polyisocyanate (3). Specific examples of the groups including the active hydrogen include a hydroxyl group (an alcoholic hydroxyl group and a phenolic hydroxyl group), an amino group, a carboxyl group, a mercapto group, etc. In particular, the alcoholic hydroxyl group is preferably used.

As the polyol (1) , diol (1-1) and polyol having 3 valences or more (1-2) can be used, and an hydrides of (1-1) alone or a mixture of (1-1) and a small amount of (1-2) are preferably used.

Specific examples of diol (1-1) include alkylene glycol such as ethylene glycol, 1,2-propylene glycol, 1,3-propylene glycol, 1,4-butanediol, and 1,6-hexanediol; alkylene ether glycol such as diethylene glycol, triethylene glycol, dipropylene glycol, polyethylene glycol, polypropylene glycol and polytetramethylene ether glycol; alicyclic diol such as 1,4-cyclohexanedimethanol and hydrogenated bisphenol A; bisphenol such as bisphenol A, bisphenol F and bisphenol S; adducts of the above-mentioned alicyclic diol with an alkylene oxide such as ethylene oxide, propylene oxide and butylene oxide; and adducts of the above-mentioned bisphenol with an alkylene oxide such as ethylene oxide, propylene oxide and butylene oxide. In particular, alkylene glycol having 2 to 12 carbon atoms and adducts of bisphenol with an alkylene oxide are preferably used, and a mixture thereof is more preferably used.

Specific examples of the polyol having 3 valences or more (1-2) include multivalent aliphatic alcohol having 3 to 8 or more valences such as glycerin, trimethylolethane, trimethylolpropane, pentaerythritol and sorbitol; phenol having 3 or more valences such as trisphenol PA, phenolnovolak, cresolnovolak; and adducts of the above-mentioned polyphenol having 3 or more valences with an alkylene oxide.

As the polycarboxylic acid (2), dicarboxylic acid (2-1) and polycarboxylic acid having 3 or more valences (2-2) can be used. (2-1) alone, or a mixture of (2-1) and a small amount of (2-2) are preferably used.

Specific examples of the dicarboxylic acid (2-1) include alkylene dicarboxylic acids such as succinic acid, adipic acid and sebacic acid; alkenylene dicarboxylic acid such as maleic acid and fumaric acid; and aromatic dicarboxylic acids such as phthalic acid, isophthalic acid, terephthalic acid and naphthalene dicarboxylic acid. In particular, alkenylene dicarboxylic acid having 4 to 20 carbon atoms and aromatic dicarboxylic acid having 8 to 20 carbon atoms are preferably used.

Specific examples of the polycarboxylic acid having 3 or more valences (2-2) include aromatic polycarboxylic acids having 9 to 20 carbon atoms such as trimellitic acid and pyromellitic acid.

The polycarboxylic acid (2) can be formed from a reaction between the polyol (1) and anhydrides of the above-mentioned acids or lower alkyl ester such as methyl ester, ethyl ester and isopropyl ester.

The polyol (1) and polycarboxylic acid (2) are mixed such that an equivalent ratio ( [OH] / [COOH] ) between a hydroxyl group [OH] and a carboxylic group [COOH] is typically from 2/1 to 1/1, preferably from 1.5/1 to 1/1, and more preferably from 1.3/1 to 1.02/1.

Specific examples of the polyisocyanate (3) include aliphatic polyisocyanate such as tetramethylenediisocyanate, hexamethylenediisocyanate and 2,6-diisocyanatemethylcaproate; alicyclicpolyisocyanate such as isophoronediisocyanate and cyclohexylmethanediisocyanate; aromatic diisocyanate such as tolylenediisocyanate and diphenylmethanediisocyanate; aromatic aliphatic diisocyanate such as α, α, α', α'-tetramethylxylylenediisocyanate; isocyanurate; the above-mentioned polyisocyanate blocked with phenol derivatives, oxime and caprolactam; and their combinations.

The polyisocyanate (3) is mixed with polyester such that an equivalent ratio ( [NCO] / [OH] ) between an isocyanate group [NCO] and polyester having a hydroxyl group [OH] is typically from 5/1 to 1/1, preferably from 4/1 to 1.2/1 and more preferably from 2.5/1 to 1.5/1. When [NCO] / [OH] is greater than 5, low-temperature fixability of the resultant toner deteriorates. When [NCO] has a molar ratio less than 1, a urea content in ester of the modified polyester decreases and hot offset resistance of the resultant toner deteriorates.

A content of the constitutional component of a polyisocyanate in the polyester prepolymer (A) having a polyisocyanate group at its end is from 0.5 to 40 % by weight, preferably from 1 to 30 % by weight and more preferably from 2 to 20 % by weight. When the content is less than 0.5 % by weight, hot offset resistance of the resultant toner deteriorates, and in addition, the heat resistance and low-temperature fixability of the toner also deteriorate. In contrast, when the content is greater than 40 % by weight, low-temperature fixability of the resultant toner deteriorates.

The number of the isocyanate groups included in a molecule of the polyester prepolymer (A) is at least 1, preferably from 1.5 to 3 on average, and more preferably from 1.8 to 2.5 on average. When the number of the isocyanate group is less than 1 per 1 molecule, the molecular weight of the modified polyester (i) decreases and hot offset resistance of the resultant toner deteriorates.

Specific examples of the amines (B) include diamines (B1), polyamines (B2) having three or more amino groups, amino alcohols (B3) , amino mercaptans (B4) , amino acids (B5) and blocked amines (B6) in which the amino groups in the amines (B1) to (B5) are blocked.

Specific examples of the diamines (B1) include aromatic diamines such as phenylene diamine, diethyltoluene diamine and 4,4'-diaminodiphenyl methane; alicyclic diamines such as 4,4'-diamino-3,3'-dimethyldicyclohexyl methane, diaminocyclohexane and isophoronediamine; aliphatic diamines such as ethylene diamine, tetramethylene diamine and hexamethylene diamine, etc.

Specific examples of the polyamines (B2) having three or more amino groups include diethylene triamine, triethylene tetramine.

Specific examples of the amino alcohols (B3) include ethanol amine and hydroxyethyl aniline.

Specific examples of the amino mercaptan (B4) include aminoethyl mercaptan and aminopropyl mercaptan.

Specific examples of the amino acids (B5) include amino propionic acid and amino caproic acid.

Specific examples of the blocked amines (B6) include ketimine compounds which are prepared by reacting one of the amines (B1) to (B5) with a ketone such as acetone, methyl ethyl ketone and methyl isobutyl ketone; oxazoline compounds, etc. Among these amines (B), diamines (B1) and mixtures in which a diamine is mixed with a small amount of a polyamine (B2) are preferably used.

A molecular weight of the modified polyesters (i) can optionally be controlled using an elongation anticatalyst, if desired. Specific examples of the elongation anticatalyst include monoamines such as diethyle amine, dibutyl amine, butyl amine and lauryl amine, and blocked amines, i.e., ketimine compounds prepared by blocking the monoamines mentioned above.

A mixing ratio (i.e., a ratio [NCO]/[NHx]) of the content of the prepolymer (A) having an isocyanate group to the amine (B) is from 1/2 to 2/1, preferably from 1.5/1 to 1/1.5 and more preferably from 1.2/1 to 1/1.2. When the mixing ratio is greater than 2 or less than 1/2, molecular weight of the urea-modified polyester (i) decreases, resulting in deterioration of hot offset resistance of the resultant toner. The modified polyester (i) may include an urethane bonding as well as a urea bonding. A molar ratio (urea/urethane) of the urea bonding to the urethane bonding is from 100/0 to 10/90, preferably from 80/20 to 20/80 and more preferably from 60/40 to 30/70. When the content of the urea bonding is less than 10 %, hot offset resistance of the resultant toner deteriorates.

The modified polyester resin (i) of the present invention can be produced by a method such as a one-shot method. The weight-average molecular weight of the modified polyester resin (i) is not less than 10, 000, preferably from 20, 000 to 10, 000, 000 and more preferably from 30,000 to 1,000,000. When the weight-average molecular weight is less than 10, 000, hot offset resistance of the resultant toner deteriorates. The number-average molecular weight of the modified polyester resin (i) is not particularly limited when the after-mentioned unmodified polyester resin (LL) is used in combination. Namely, the weight-average molecular weight of the modified polyester resin (i) has priority over the number-average molecular weight thereof. However, when the modified polyester resin (i) is used alone, the number-average molecular weight is from 2,000 to 15, 000, preferably from 2, 000 to 10, 000 and more preferably from 2,000 to 8,000. When the number-average molecular weight is greater than 20,000, a low-temperature fixability of the resultant toner deteriorates, and in addition a glossiness of full color images deteriorates.

### Unmodified polyester resin (LL)

In the present invention, an unmodified polyester resin (LL) can be used in combination with the modified polyester resin (i) as a toner binder resin. It is more preferable to use the unmodified polyester resin (LL) in combination with the modified polyester resin than to use the modified polyester resin alone because a low-temperature fixability and a glossiness of full color images of the resultant toner improve. Specific examples of the unmodified polyester resin (LL) include polycondensated products between the polyol (1) and polycarboxylic acid (2) similarly to the modified polyester resin (i), and products preferably used are the same as those thereof. It is preferable that the modified polyester resin (i) and unmodified polyester resin (LL) are partially soluble in each other in terms of the low-temperature fixability and hot offset resistance of the resultant toner. Therefore, the modified polyester resin (i) and unmodified polyester resin (LL) preferably have similar compositions. When the unmodified polyester resin (LL) is used in combination, a weight ratio ( (i) / (LL) ) between the modified polyester resin (i) and unmodified polyester resin (LL) is from 5/95 to 80/20, preferably from 5/95 to 30/70, more preferably from 5-95 to 25/75, and most preferably from 7/93 to 20/80. When the modified polyester resin (i) has a weight ratio less than 5 %, hot offset resistance the resultant toner deteriorates, and has a difficulty in having a thermostable preservability and a low-temperature fixability deteriorate.

The unmodified polyester resin (LL) preferably has a peak molecular weight of from 1, 000 to 20, 000, preferably from 1, 500 to 10, 000, and more preferably from 2, 000 to 8, 000. When less than 1,000, the thermostable preservability of the resultant toner deteriorates. When greater than 10,000, the low-temperature fixability thereof deteriorates. The unmodified polyester resin (LL) preferably has a an acid value not less than 5 mg KOH/g, more preferably of from 10 to 120 mg KOH/g, and most preferably from 20 to 80 mg KOH/g. When less than 5, the resultant toner has a difficulty in having a thermostable preservability and a low-temperature fixability. The unmodified polyester resin (LL) preferably has an acid value of from 10 to 30 mg KOH/g such that the resultant toner tends to be negatively charged and to have better fixability. When greater than 30 mg KOH/g, chargeability of the resultant toner deteriorates when particularly used in an environment of high humidity and high temperature, and may produce images having background fouling.

In the present invention, the unmodified polyester resin (LL) preferably has a glass transition temperature (Tg) of from 35 to 55 °C, and more preferably from 40 to 55 °C. The resultant toner can have a thermostable preservability and a low-temperature fixability. A dry toner of the present invention including the unmodified polyester resin (LL) and the modified polyester resin (i) has a better thermostable preservability than known polyester toners even though the glass transition temperature is low.

In the present invention, thetonerbinderresinpreferably has a temperature (TG' ) not less than 100°C, and more preferably of from 110 to 200 °C at which a storage modulus of the toner binder resin is 10,000 dyne/cm² at a measuring frequency of 20 Hz. When less than 100 °C, the hot offset resistance of the resultant toner deteriorates. The toner binder resin preferably has a temperature (T η) not greater than 180 °C, and more preferably of from 90 to 160 °C at which a viscosity is 1,000 poise. When greater than 180 °C, the low-temperature fixability of the resultant toner deteriorates. Namely, TG' is preferably higher than T η in terms of the low-temperature fixability and hot offset resistance of the resultant toner. In other words, a difference between TG' and T η (TG'-Tη) is preferably not less than 0 °C, more preferably not less than 10 °C, and furthermore preferably not less than 20 °C . A maximum of the difference is not particularly limited. In terms of the thermostable preservability and low-temperature fixability of the resultant toner, the difference between TG' and T η (TG' -T η) is preferably from 0 to 20 °C, more preferably from 10 to 90 °C, and most preferably from 20 to 80 °C.

Specific examples of the colorants for use in the present invention include any known dyes and pigments such as carbon black, Nigrosine dyes, black iron oxide, Naphthol Yellow S, Hansa Yellow (10G, 5G and G) , Cadmium Yellow, yellow iron oxide, loess, chrome yellow, Titan Yellow, polyazo yellow, Oil Yellow, Hansa Yellow (GR, A, RN and R), Pigment Yellow L, Benzidine Yellow (G and GR), Permanent Yellow (NCG), Vulcan Fast Yellow (5G and R), Tartrazine Lake, Quinoline Yellow Lake, Anthrazane Yellow BGL, isoindolinone yellow, red iron oxide, red lead, orange lead, cadmium red, cadmium mercury red, antimony orange, Permanent Red 4R, Para Red, Fire Red, p-chloro-o-nitroaniline red, Lithol Fast Scarlet G, Brilliant Fast Scarlet, Brilliant Carmine BS, Permanent Red (F2R, F4R, FRL, FRLL and F4RH) , Fast Scarlet VD, Vulcan Fast Rubine B, Brilliant Scarlet G, Lithol Rubine GX, Permanent Red F5R, Brilliant Carmine 6B, Pigment Scarlet 3B, Bordeaux 5B, Toluidine Maroon, Permanent Bordeaux F2K, Helio Bordeaux BL, Bordeaux 10B, BON Maroon Light, BON Maroon Medium, Eosin Lake, Rhodamine Lake B, Rhodamine Lake Y, Alizarine Lake, Thioindigo Red B, Thioindigo Maroon, Oil Red, Quinacridone Red, Pyrazolone Red, polyazored, Chrome Vermilion, Benzidine Orange, perynone orange, Oil Orange, cobalt blue, cerulean blue, Alkali Blue Lake, Peacock Blue Lake, Victoria Blue Lake, metal-free Phthalocyanine Blue, Phthalocyanine Blue, Fast Sky Blue, IndanthreneBlue (RSandBC) , Indigo, ultramarine, Prussianblue, Anthraquinone Blue, Fast Violet B, Methyl Violet Lake, cobalt violet, manganese violet, dioxane violet, Anthraquinone Violet, Chrome Green, zinc green, chromiumoxide, viridian, emeraldgreen, Pigment Green B, Naphthol Green B, Green Gold, Acid Green Lake, Malachite Green Lake, Phthalocyanine Green, Anthraquinone Green, titanium oxide, zinc oxide, lithopone and the like. These materials are used alone or in combination.

A content of the colorant in the toner is preferably from 1 to 15 % by weight, and more preferably from 3 to 10 % by weight, based on total weight of the toner.

The colorant for use in the present invention can be used as a master batch pigment when combined with a resin.

Specific examples of the resin for use in the master batch pigment or for use in combination with master batch pigment include the modified and unmodified polyester resins mentioned above; styrene polymers and substituted styrene polymers such as polystyrene, poly-p-chlorostyrene and polyvinyltoluene; styrene copolymers such as styrene-p-chlorostyrene copolymers, styrene-propylene copolymers, styrene-vinyltoluene copolymers, styrene-vinylnaphthalene copolymers, styrene-methyl acrylate copolymers, styrene-ethyl acrylate copolymers, styrene-butyl acrylate copolymers, styrene-octyl acrylate copolymers, styrene-methyl methacrylate copolymers, styrene-ethyl methacrylate copolymers, styrene-butyl methacrylate copolymers, styrene-methyl α-chloromethacrylate copolymers, styrene-acrylonitrile copolymers, styrene-vinyl methyl ketone copolymers, styrene-butadiene copolymers, styrene-isoprene copolymers, styrene-acrylonitrile-indene copolymers, styrene-maleic acid copolymers and styrene-maleic acid ester copolymers; and other resins such as polymethyl methacrylate, polybutylmethacrylate, polyvinyl chloride, polyvinyl acetate, polyethylene, polypropylene, polyesters, epoxy resins, epoxy polyol resins, polyurethane resins, polyamide resins, polyvinyl butyral resins, acrylic resins, rosin, modified rosins, terpene resins, aliphatic or alicyclic hydrocarbon resins, aromatic petroleum resins, chlorinated paraffin, paraffin waxes, etc. These resins are used alone or in combination.

The master batch for use in the toner of the present invention is typically prepared by mixing and kneading a resin and a colorant upon application of high shear stress thereto. In this case, an organic solvent can be used to heighten the interaction of the colorant with the resin. In addition, flushing methods in which an aqueous paste including a colorant is mixed with a resin solution of an organic solvent to transfer the colorant to the resin solution and then the aqueous liquid and organic solvent are separated and removed can be preferably used because the resultant wet cake of the colorant can be used as it is. Of course, a dry powder which is prepared by drying the wet cake can also be used as a colorant. In this case, a three roll mill is preferably used for kneading the mixture upon application of high shearing stress.

The toner of the present invention may include a wax together with a binder resin and a colorant. A status of presence of the wax in a toner largely affects releasability thereof when fixed, and when the wax is finely dispersed in a toner and present close to the surface thereof in a large amount, the toner has good releasability. Particularly, the wax is preferably dispersed with a major axis not greater than 1 µm. When the wax is present on the surface of the toner in a large amount, the wax is easily released therefromwhen stirred for long periods in an image developer and adhered to the surface of a carrier and a member of the image developer, resulting in deterioration of chargeability of a developer including the toner.

The dispersion status of the wax is observed with an amplified picture taken through a transmission electron microscope.

Specific examples of the wax include known waxes, e.g., polyolef in waxes such as polyethylene wax and polypropylene wax; long chain carbon hydrides such as paraffin wax and sasol wax; and waxes including carbonyl groups. Among these waxes, the waxes including carbonyl groups are preferably used. Specific examples thereof include polyesteralkanate such as carnauba wax, montan wax, trimethylolpropanetribehenate, pentaerythritoltetrabehenate, pentaerythritoldiacetatedibehenate, glycerinetribehenate and 1,18-octadecanedioldistearate; polyalkanolesters such as tristearyltrimellitate and distearylmaleate; polyamidealkanate such as ethylenediaminebehenylamide; polyalkylamide such as tristearylamidetrimellitate; and dialkylketone such as distearylketone. Among these waxes including a carbonyl group, polyesteralkanate is preferably used.

The wax for use in the present invention usually has a melting point of from 40 to 160 °C, preferably of from 50 to 120°C, and more preferably of from 60 to 90 °C. A wax having a melting point less than 40 °C has an adverse effect on its high temperature preservability, and a wax having a melting point greater than 160 °C tends to cause cold offset of the resultant toner when fixed at a low temperature. In addition, the wax preferably has a melting viscosity of from 5 to 1,000 cps, and more preferably of from 10 to 100 cps when measured at a temperature higher than the melting point by 20 °C. A wax having a melting viscosity greater than 1, 000 cps may make it difficult to improve hot offset resistance and low temperature fixability of the resultant toner. A content of the wax in a toner is preferably from 0 to 40 % by weight, and more preferably from 3 to 30 % by weight.

The toner of the present invention may optionally include a charge controlling agent. The charge controlling agent fixed on the toner surface can improve chargeability of the toner. When the charge controlling agent is fixed on the toner surface, a presence amount and status thereof can be stabilized, and therefore the chargeability of the toner can be stabilized. Particularly, the toner of the present invention has better chargeability when including the charge controlling agent.

Specific examples of the charge controlling agent include any known charge controlling agents such as Nigrosine dyes, triphenylmethane dyes, metal complex dyes including chromium, chelate compounds of molybdic acid, Rhodamine dyes, alkoxyamines, quaternary ammonium salts (including fluorine-modified quaternary ammonium salts) , alkylamides, phosphor and compounds including phosphor, tungsten and compounds including tungsten, fluorine-containing activators, metal salts of salicylic acid, salicylic acid derivatives, etc.

Specific examples of the marketed products of the charge controlling agents include BONTRON 03 (Nigrosine dyes) , BONTRON P-51 (quaternary ammonium salt),BONTRON S-34 (metal-containing azo dye) , E-82 (metal complex of oxynaphthoic acid) , E-84 (metal complex of salicylic acid), and E-89 (phenolic condensation product) , which are manufactured by Orient Chemical Industries Co., Ltd.; TP-302 and TP-415 (molybdenum complex of quaternary ammoniumsalt) , which are manufactured by Hodogaya Chemical Co., Ltd.; COPY CHARGE PSY VP2038 (quaternary ammonium salt) , COPY BLUE (triphenyl methane derivative) , COPY CHARGE NEG VP2036 and NX VP434 (quaternary ammonium salt) , which are manufactured by Hoechst AG; LRA-901, and LR-147 (boron complex), which are manufactured by Japan Carlit Co., Ltd.; copper phthalocyanine, perylene, quinacridone, azo pigments and polymers having a functional group such as a sulfonate group, a carboxyl group, a quaternary ammonium group, etc.

A content of the charge controlling agent is determined depending on the species of the binder resin used, whether or not an additive is added and toner manufacturing method (such as dispersion method) used, and is not particularly limited. However, the content of the charge controlling agent is typically from 0.1 to 10 parts by weight, and preferably from 0.2 to 5 parts by weight, per 100 parts by weight of the binder resin included in the toner. When the content is too high, the toner may have too large charge quantity, and thereby the electrostatic force of a developing roller attracting the toner increases, resulting in deterioration of the fluidity of the toner and image density of the toner images.

These charge controlling agent and release agent can be kneaded upon application of heat together with a master batch pigment and a resin, or can be added to toner constituents when dissolved and dispersed in an organic solvent.

The toner of the present invention may include a cleanability improver for removing a developer remaining on a photoreceptor and a first transfer medium after transferred. Specific examples of the cleanability improver include fatty acid metallic salts such as zinc stearate, calcium stearate and stearic acid; and polymer particles prepared by a soap-free emulsifying polymerization method such as polymethylmethacrylate particles and polystyrene particles. The polymer particles comparatively have a narrow particle diameter distribution and preferably. have a volume-average particle diameter of from 0.01 to 1 µm.

The toner binder of the present invention can be prepared, for example, by the following method. Polyol (1) and polycarboxylic acid (2) are heated at a temperature of from 150 to 280 °C in the presence of a known catalyst such as tetrabutoxy titanate and dibutyltinoxide. Then water generated is removed, under a reduced pressure if desired, to prepare a polyester resin having a hydroxyl group. Then the polyester resin is reacted with polyisocyanate (3) at a temperature of from 40 to 140 °C to prepare a prepolymer (A) having an isocyanate group. Further, the prepolymer (A) is reacted with an amine (B) at a temperature of from 0 to 140 °C, to prepare a modified polyester resin (i). When polyisocyanate, and A and B are reacted, a solvent can be used if desired. Suitable solvents include solvents which do not react with polyisocyanate (3). Specific examples of such solvents include aromatic solvents such as toluene and xylene; ketones such as acetone, methyl ethyl ketone and methyl isobutyl ketone; esters such as ethyl acetate; amides such as dimethylformamide and dimethylacetoamide; ethers such as tetrahydrofuran.

When polyester (LL) which does not have a urea bonding is used in combination with the urea-modified polyester, a method similar to a method for preparing a polyester resin having a hydroxyl group is used to prepare the polyester resin (LL) which does not have a urea bonding, and the polyester (LL) which does not have a urea bonding is dissolved and mixed in a solution after a reaction of the modified polyester (i) is completed.

A dry toner is produced by the following method, but the method is not limited thereto.

Toner constituents such as a toner binder resin including the modified polyester resin (i), a charge controlling agent and a pigment are mechanically mixed. This mixing process can be performed with an ordinary mixer such as rotating blades under ordinary conditions, and is not particularly limited.

After the mixing process is completed, the mixture is kneaded upon application of heat by a kneader. The kneader includes axial and biaxial continuous kneaders, and roll-mill batch type kneaders. It is essential to see that the kneading upon application of heat does not cut a molecular chain of the toner binder resin. Specifically, the kneading temperature depends on a softening point of the toner binder resin. When too lower than the softening point, cutting of the molecular chain of the toner binder resin increases. When too higher than the softening point, the toner binder resin is not well dispersed.

After the kneading process is completed, the kneaded mixture is pulverized. The mixture is preferably crushed first, and next pulverized. Methods of crushing the mixture to a collision board and pulverizing the mixture in a narrow gap between a rotor and a stator mechanically rotated are preferably used.

After the pulverizingprocess is completed, the pulverized mixture is classified in an airstream by a centrifugal force to prepare a toner having a predetermined particle diameter, e.g., an average particle diameter of from 5 to 20 µm.

In addition, to improve the fluidity, preservability, developability and transferability of the toner, the inorganic fine particles such as a hydrophobic silica fine powder as mentioned above is externally added to the toner. A conventional powder mixer can be used to mix the external additive, and the mixer preferably has a jacket and can control an inner temperature thereof. To change a history of a load to the external additive, the external additive may be added to the toner completely prior to mixing or gradually added thereto during mixing. As a matter of course, the number of revolutions, a rolling speed, a time and a temperature of the mixer may be changed. A large load first and next a small load, or vice versa may be applied to the toner.

Specific examples of the mixer include a V-form mixer, a locking mixer, a Loedige Mixer, a Nauter Mixer, a Henshel Mixer, etc.

To ensphere the toner, many methods can be used, including a method of mechanically ensphering the toner by using a hybridizer or a Mechanofusion after the pulverizing process, a method which is a so-called spray dry method of ensphering the toner by using a spray dryer to remove a solvent after toner materials are dissolved and dispersed in the solvent capable of dissolving a toner binder, and a method of ensphering the toner by heating the toner in an aqueous medium. However, the methods are not limited thereto.

The toner of the present invention may be prepared by the following method.

First, an oil dispersion wherein a polyester prepolymer including an isocyanate group A is dissolved in an organic solvent, a colorant is dispersed and a release agent is dissolved or dispersed is prepared.

The oil dispersion is pulverized by a wet pulverizer to pulverize and uniformly disperse the colorant therein for 30 to 120 min.

Next, the oil dispersion is emulsified in the presence of an inorganic particulate material and/or a particulate polymer material to form an oil-in-water emulsion and a urea-modified polyester resin C produced by a reaction between the polyester prepolymer including an isocyanate group A and an amine B.

Specific examples of the organic solvent include organic solvents dissolving polyester resins, and which is insoluble, hardly soluble or slightly soluble in water. The organic solvent preferably has a boiling point of from 60 to 150 °C, and more preferably from 70 to 120°C. Specific examples of such an organic solvent include ethyl acetate, methyl ethyl ketone, etc.

A solid particulate dispersant in the aqueous phase uniformly disperses oilspots therein. The solid particulate dispersant is located on a surface of the oilspot, and the oilspots are uniformly dispersed and an assimilation among the oilspots is prevented. Therefore, the resultant toner has a sharp particle diameter distribution.

The solid particulate dispersant is preferably an inorganic particulate material having an average particle diameter of from 0.01 to 1 µm, which is difficult to dissolve in water and is solid in the aqueous medium.

Specific examples of the inorganic particulate material include silica, alumina, titanium oxide, barium titanate, magnesium titanate, calcium titanate, strontium titanate, zinc oxide, tin oxide, quartz sand, clay, mica, sand-lime, diatom earth, chromium oxide, cerium oxide, red iron oxide, antimony trioxide, magnesium oxide, zirconium oxide, barium sulfate, barium carbonate, calcium carbonate, silicon carbide, silicon nitride, etc.

Further, tricalcium phosphate, calcium carbonate, colloidal titanium oxide, colloidal silica and hydroxyapatite are preferably used. Particularly, the hydroxyapatite which is a basic reaction product between sodium phosphate and calcium chloride is more preferably used.

The dispersion method is not particularly limited, and low speed shearing methods, high-speed shearing methods, friction methods, high-pressure jet methods, ultrasonic methods, etc. can be used. Among these methods, high-speed shearing methods are preferably used because particles having a particle diameter of from 2 to 20 µm can be easily prepared. At this point, the particle diameter (2 to 20 µm) means a particle diameter of particles including a liquid). When a high-speed shearing type dispersion machine is used, the rotation speed is not particularly limited, but the rotation speed is typically from 1,000 to 30,000 rpm, and preferably from 5,000 to 20,000 rpm. The dispersion time is not also particularly limited, but is typically from 0.1 to 5 minutes. The temperature in the dispersion process is typically from 0 to 150 °C (under pressure), and preferably from 40 to 98 °C. When the temperature is relatively high, the modified polyester (i) or prepolymer (A) can easily be dispersed because the dispersion formed has a low viscosity.

A content of the aqueous medium to 100 parts by weight of the toner constituents including the modified polyester (i) or prepolymer (A) is typically from 50 to 2, 000 parts by weight, and preferably from 100 to 1,000 parts by weight. When the content is less than 50 parts by weight, the dispersion of the toner constituents in the aqueous medium is not satisfactory, and thereby the resultant mother toner particles do not have a desired particle diameter. In contrast, when the content is greater than 2,000, the production cost increases. A dispersant can preferably be used to prepare a stably dispersed dispersion including particles having a sharp particle diameter distribution.

Specific examples of the dispersants used to emulsify and disperse an oil phase for a liquid including water in which the toner constituents are dispersed include anionic surfactants such as alkylbenzene sulfonic acid salts, α-olefin sulfonic acid salts, and phosphoric acid salts; cationic surfactants such as amine salts (e.g., alkyl amine salts, aminoalcohol fatty acid derivatives, polyamine fatty acid derivatives and imidazoline), and quaternary ammonium salts (e.g., alkyltrimethyl ammonium salts, dialkyldimethyl ammonium salts, alkyldimethyl benzyl ammonium salts, pyridinium salts, alkyl isoquinolinium salts and benzethonium chloride) ; nonionic surfactants such as fatty acid amide derivatives, polyhydric alcohol derivatives; and ampholytic surfactants such as alanine, dodecyldi(aminoethyl)glycin, di(octylaminoethyl)glycin, and N-alkyl-N,N-dimethylammonium betaine.

A surfactant having a fluoroalkyl group can be used to prepare a dispersion having good dispersibility even when a small amount of the surfactant is used. Specific examples of anionic surfactants having a fluoroalkyl group include fluoroalkyl carboxylic acids having from 2 to 10 carbon atoms and their metal salts, disodium perfluorooctanesulfonylglutamate, sodium 3-{omega-fluoroalkyl (C6-C11) oxy}-1-alkyl (C3-C4) sulfonate, sodium- {omega-fluoroalkanoyl (C6-C8)-N-ethylamino}-1-propanesulfonate, fluoroalkyl (C11-C20) carboxylic acids and their metal salts, perfluoroalkylcarboxylic acids and their metal salts, perfluoroalkyl (C4-C12) sulfonate and their metal salts, perfluorooctanesulfonic acid diethanol amides, N-propyl-N-(2-hydroxyethyl)perfluorooctanesulfone amide, perfluoroalkyl(C6-C10)sulfoneamidepropyltrimethylammonium salts, salts of perfluoroalkyl(C6-C10)-N-ethylsulfonylglycin, monoperfluoroalkyl(C6-C16)ethylphosphates, etc.

Specific examples of the marketed products of such surfactants having a fluoroalkyl group include SURFLON S-111, S-112 and S-113, which are manufactured by Asahi Glass Co., Ltd.; FRORARD FC-93, FC-95, FC-98 and FC-129, which are manufactured by Sumitomo 3M Ltd.; UNIDYNE DS-101 and DS-102, which are manufactured by Daikin Industries, Ltd.;MEGAFACEF-110, F-120, F-113, F-191, F-812 and F-833 which are manufactured by Dainippon Ink and Chemicals, Inc.; ECTOP EF-102, 103, 104, 105, 112, 123A, 306A, 501, 201 and 204, which are manufactured by Tohchem Products Co., Ltd. ; FUTARGENT F-100 and F150 manufactured by Neos; etc.

Specific examples of the cationic surfactants, which can disperse an oil phase including toner constituents in water, include primary, secondary and tertiary aliphatic amines having a fluoroalkyl group, aliphatic quaternary ammonium salts such as erfluoroalkyl (C6-C10)sulfoneamidepropyltrimethylammonium salts, benzalkonium salts, benzetonium chloride, pyridinium salts, imidazolinium salts, etc. Specific examples of the marketed products thereof include SURFLONS-121 (fromAsahiGlass Co., Ltd.); FRORARD FC-135 (from Sumitomo 3M Ltd.); UNIDYNE DS-202 (from Daikin Industries, Ltd.) ; MEGAFACE F-150 and F-824 (from Dainippon Ink and Chemicals, Inc.); ECTOP EF-132 (from Tohchem Products Co., Ltd.) ; FUTARGENT F-300 (from Neos) ; etc.

In addition, inorganic compound dispersants such as tricalcium phosphate, calcium carbonate, titanium oxide, colloidal silica and hydroxyapatite which are hardly insoluble in water can also be used.

Further, it is possible to stably disperse toner constituents in water using a polymeric protection colloid. Specific examples of such protection colloids include polymers and copolymers prepared using monomers such as acids (e.g., acrylic acid, methacrylic acid, α-cyanoacrylic acid, α -cyanomethacrylic acid, itaconic acid, crotonic acid, fumaric acid, maleic acid and maleic anhydride) , acrylic monomers having a hydroxyl group (e.g., β-hydroxyethyl acrylate, β -hydroxyethyl methacrylate, β-hydroxypropyl acrylate, β -hydroxypropyl methacrylate, γ-hydroxypropyl acrylate, γ -hydroxypropyl methacrylate, 3-chloro-2-hydroxypropyl acrylate, 3-chloro-2-hydroxypropyl methacrylate, diethyleneglycolmonoacrylic acid esters, diethyleneglycolmonomethacrylic acid esters, glycerinmonoacrylic acid esters, N-methylolacrylamide and N-methylolmethacrylamide) , vinyl alcohol and its ethers (e.g. , vinyl methyl ether, vinyl ethyl ether and vinyl propyl ether) , esters of vinyl alcohol with a compound having a carboxyl group (i.e., vinyl acetate, vinyl propionate and vinyl butyrate); acrylic amides (e.g, acrylamide, methacrylamide and diacetoneacrylamide) and their methylol compounds, acid chlorides (e.g., acrylic acid chloride and methacrylic acid chloride) , and monomers having a nitrogen atom or an alicyclic ring having a nitrogen atom (e.g., vinyl pyridine, vinyl pyrrolidone, vinyl imidazole and ethylene imine). In addition, polymers such as polyoxyethylene compounds (e.g., polyoxyethylene, polyoxypropylene, polyoxyethylenealkyl amines, polyoxypropylenealkyl amines, polyoxyethylenealkyl amides, polyoxypropylenealkyl amides, polyoxyethylene nonylphenyl ethers, polyoxyethylene laurylphenyl ethers, polyoxyethylene stearylphenyl esters, and polyoxyethylene nonylphenyl esters); and cellulose compounds such as methyl cellulose, hydroxyethyl cellulose and hydroxypropyl cellulose, can also be used as the polymeric protective colloid.

When an acid such as calciumphosphate or a material soluble in alkali is used as a dispersant, the calcium phosphate is dissolved with an acid such as a hydrochloric acid and washed with water to remove the calcium phosphate from the toner particle. Besides this method, it can also be removed by an enzymatic hydrolysis.

When a dispersant is used, the dispersant may remain on a surface of the toner particle. However, the dispersant is preferably washed and removed after the elongation and/or crosslinking reaction of the prepolymer with amine.

Further, to decrease viscosity of a dispersion medium including the toner constituents, a solvent which can dissolve the modified polyester (i) or prepolymer (A) can be used because the resultant particles have a sharp particle diameter distribution. The solvent is preferably volatile and has a boiling point lower than 100 °C because of easily removed from the dispersion after the particles are formed. Specific examples of such a solvent include toluene, xylene, benzene, carbon tetrachloride, methylene chloride, 1,2-dichloroethane, 1,1,2-trichloroethane, trichloroethylene, chloroform, monochlorobenzene, dichloroethylidene, methyl acetate, ethyl acetate, methyl ethyl ketone, methyl isobutyl ketone, etc. These solvents can be used alone or in combination. Among these solvents, aromatic solvents such as toluene and xylene; and halogenated hydrocarbons such as methylene chloride, 1,2-dichloroethane, chloroform, and carbon tetrachloride are preferably used.

The addition quantity of such a solvent is from 0 to 300 parts by weight, preferably from 0 to 100, and more preferably from 25 to 70 parts by weight, per 100 parts by weight of the prepolymer (A) used. When such a solvent is used to prepare a particle dispersion, the solvent is removed therefrom under a normal or reduced pressure after the particles are subjected to an elongation reaction and/or a crosslinking reaction of the prepolymer with amine.

The elongation and/or crosslinking reaction time depend on reactivity of an isocyanate structure of the prepolymer (A) and amine (B), but is typically from 10 min to 40 hrs, and preferably from 2 to 24 hrs. The reaction temperature is typically from 0 to 150 °C, and preferably from 40 to 98 °C. In addition, a known catalyst such as dibutyltinlaurate and dioctyltinlaurate can be used.

To remove an organic solvent from the emulsified dispersion, a method of gradually raising a temperature of the whole dispersion to completely remove the organic solvent in the droplet by vaporizing can be used. Otherwise, a method of spraying the emulsified dispersion in a dry air, completely removing a water-insoluble organic solvent in the droplet to form toner particles and removing a water dispersant by vaporizing can also be used. As the dry air, an atmospheric air, a nitrogen gas, carbon dioxide gas, a gaseous body in which a combustion gas is heated, and particularly various aerial currents heated to have a temperature not less than a boiling point of a solvent used are typically used. A spray dryer, a belt dryer and a rotary kiln can sufficiently remove the organic solvent in a short time.

When the emulsified dispersion is washed and dried while maintaining a wide particle diameter distribution thereof, the dispersion can be classified to have a desired particle diameter distribution.

A cyclone, a decanter, a centrifugal separation, etc. can remove particles in a dispersion liquid. A powder after the dispersion liquid is dried can be classified, but the liquid is preferably classified in terms of efficiency. Unnecessary fine and coarse particles can be recycled to a kneading process to form particles. The fine and coarse particles may be wet when recycled.

A dispersant is preferably removed from a dispersion liquid, and more preferably removed at the same time when the above-mentioned classification is performed.

Heterogeneous particles such as release agent particles, charge controlling particles, fluidizing particles and colorant particles can be mixed with a toner powder after dried. Release of the heterogeneous particles from composite particles can be prevented by giving a mechanical stress to a mixed powder to fix and fuse them on a surface of the composite particles.

Specific methods include a method of applying an impact strength on a mixture with a blade rotating at a high-speed, a method of putting a mixture in a high-speed stream and accelerating the mixture such that particles thereof collide each other or composite particles thereof collide with a collision board, etc. Specific examples of the apparatus include an ONG MILL from Hosokawa Micron Corp. , a modified I-type mill having a lower pulverizing air pressure from Nippon Pneumatic Mfg. Co., Ltd., a hybridization system from Nara Machinery Co., Ltd., a Kryptron System from Kawasaki Heavy Industries, Ltd., an automatic mortar, etc.

The toner of the present invention can be used for a two-component developer in which the toner is mixed with a magnetic carrier. A content of the toner is preferably from 1 to 10 parts by weight per 100 parts by weight of the carrier.

Suitable carriers for use in the two component developer include known carrier materials such as iron powders, ferrite powders, magnetite powders, magnetic resin carriers, which have a particle diameter of from about 20 to about 200 µm.

The carrier may be coated by a resin. Specific examples of such resins to be coated on the carriers include amino resins such as urea-formaldehyde resins, melamine resins, benzoguanamine resins, urea resins, and polyamide resins, and epoxy resins. In addition, vinyl or vinylidene resins such as acrylic resins, polymethylmethacrylate resins, polyacrylonitirile resins, polyvinyl acetate resins, polyvinyl alcohol resins, polyvinyl butyral resins, polystyrene resins, styrene-acrylic copolymers, halogenated olefin resins such as polyvinyl chloride resins, polyester resins such as polyethyleneterephthalate resins and polybutyleneterephthalate resins, polycarbonate resins, polyethylene resins, polyvinyl fluoride resins, polyvinylidene fluoride resins, polytrifluoroethylene resins, polyhexafluoropropylene resins, vinylidenefluoride-acrylate copolymers, vinylidenefluoride-vinylfluoride copolymers, copolymers of tetrafluoroethylene, vinylidenefluoride and other monomers including no fluorine atom, and silicone resins.

An electroconductive powder may optionally be included in the toner. Specific examples of such electroconductive powders include metal powders, carbon blacks, titanium oxide, tin oxide, and zinc oxide. The average particle diameter of such electroconductive powders is preferably not greater than 1 µm. When the particle diameter is too large, it is hard to control the resistance of the resultant toner.

The toner of the present invention can also be used as a one-component magnetic or non-magnetic developer without a carrier.

Amorphous silicon photoreceptors (hereinafter referred to as a-Si photoreceptors) can be used in the present invention, which is formed by heating an electroconductive substrate at from 50 to 400 °C and forming an a-Si photosensitive layer on the substrate by a vacuum deposition method, a sputtering method, an ion plating method, a heat CVD method, a photo CVD method, a plasma CVD method, etc. Particularly, the plasma CVD method is preferably used, which forms an a-Si layer on the substrate by decomposing a gas material with a DC, a high-frequency or a microwave glow discharge.

Figs. 1A to 1D are schematic views illustrating a photosensitive layer composition of the amorphous photoreceptor for use in the present invention respectively. An electrophotographic photoreceptor 500 in Fig. 1A includes a substrate 501 and a photosensitive layer 503 thereon, which is photoconductive and formed of a-Si. An electrophotographic photoreceptor 500 in Fig. 1B includes a substrate 501, a photosensitive layer 502 thereon and an a-Si surface layer 503 on the photosensitive layer 502. An electrophotographic photoreceptor 500 in Fig. 1C includes a substrate 501, a charge injection prevention layer 504 thereon, a photosensitive layer 502 on the charge injection prevention layer 504 and an a-Si surface layer 503 on the photosensitive layer 502. An electrophotographic photoreceptor 500 in Fig. 1D includes a substrate 501, a photosensitive layer 502 thereon including a charge generation layer 505 and a charge transport layer formed of a-Si, and an a-Si surface layer 503 on the photosensitive layer 502.

The substrate of the photoreceptor may either be electroconductive or insulative. Specific examples of the substrate include metals such as Al, Cr, Mo, Au, In, Nb, Te, V, Ti, Pt, Pd and Fe and their alloyed metals such as stainless steel. In addition, insulative substrates such as films or sheets of synthetic resins such as polyester, polyethylene, polycarbonate, cellulose acetate, polypropylene, polyvinylchloride, polystyrene, polyamide; glasses; and ceramics can be used, provided at least a surface of the substrate on which a photosensitive layer is formed is treated to be electroconductive. The substrate has the shape of a cylinder, a plate or an endless belt having a smooth or a concave-convex surface. The substrate can have a desired thickness, which can be as thin as possible when an electrophotographic photoreceptor including the substrate is required to have flexibility. However, the thickness is typically not less than 10 µm in terms of production and handling conveniences, and a mechanical strength of the electrophotographic photoreceptor.

The a-Si photoreceptor of the present invention may optionally include the charge injection prevention layer between the electroconductive substrate and the photosensitive layer in Fig. 3C. When the photosensitive layer is charged with a charge having a certainpolarity, the charge inj ectionprevention layer prevents a charge from being injected into the photosensitive layer from the substrate. However, the charge inj ectionprevention layer does not when the photosensitive layer is charged with a charge having a reverse polarity, i.e., has a dependency on the polarity. The charge injection prevention layer includes more atoms controlling conductivity than the photosensitive layer to have such a capability.

The charge injection prevention layer preferably has a thickness of from 0.1 to 5 µm, more preferably from 0.3 to 4 µm, and most preferably from 0.5 to 3 µm in terms of desired electrophotographic properties and economic effects. The photosensitive layer 502 is formed on an undercoat layer optionally formed on the substrate 501 and has a thickness as desired, and preferably of from 1 to 100 µm, more preferably from 20 to 50 µm, and most preferably from 23 to 45 µm in terms of desired electrophotographic properties and economic effects.

The charge transport layer is a layer transporting a charge when the photosensitive layer is functionally separated. The charge transport layer includes at least a silicon atom, a carbon atom and a fluorine atom, and optionally includes a hydrogen atom and an oxygen atom. Further, the charge transport layer has a photosensitivity, a charge retainability, a charge generation capability and a charge transportability as desired. In the present invention, the charge transport layer preferably includes an oxygen atom.

The charge transport layer has a thickness as desired in terms of electrophotographic properties and economic effects, and preferably of from 5 to 50 µm, more preferably from 10 to 40 µm, and most preferably from 20 to 30 µm.

The charge generation layer is a layer generating a charge when the photosensitive layer is functionally separated. The charge generation layer includes at least a silicon atom, substantially does not include a carbon atom and optionally includes a hydrogen atom. Further, the charge generation layer has a photosensitivity, a charge generation capability and a charge transportability as desired.

The charge generation layer has a thickness as desired in terms of electrophotographic properties and economic effects, and preferably of from 0.5 to 15 µm, more preferably from 1 to 10 µm, and most preferably from 1 to 5 µm.

The a-Si photoreceptor for use in the present invention can optionally include a surface layer on the photosensitive layer formed on the substrate, which is preferably an a -Si surface layer. The surface layer has a free surface and is formed to attain objects of the present invention in humidity resistance, repeated use resistance, electric pressure resistance, environment resistance and durability of the photoreceptor.

The surface layer preferably has a thickness of from 0.01 to 3 µm, more preferably from 0. 05 to 2 µm, and most preferably from 0.1 to 1 µm. When less than 0.01 µm, the surface layer is lost due to abrasion while the photoreceptor is used. When greater than 3 µm, deterioration of the electrophotographic properties such as an increase of residual potential of the photoreceptors occurs.

In an image developer (2) in Fig. 2, a vibration bias voltage which is a DC voltage overlapped with an AC voltage is applied to a developing sleeve (4) from an electric source (10) as a developing bias when developing an image. A background potential and an image potential are located between a maximum and a minimum of the vibration bias potential. An alternating electric field changing the direction alternately is formed at a developing portion (D). In the alternating electric field, a toner and a carrier intensely vibrate, and the toner flies to a photoreceptor drum (1) being released from an electrostatic binding force of the developing sleeve (4) and the carrier and is transferred to a latent image on the photoreceptor drum (1) .

A difference between the maximum and minimum of the vibration bias voltage (voltage between the peaks) is preferably from 0.5 to 5 KV, and a frequency thereof is preferably from 1 to 10 KHz. The vibration bias voltage can have the waveform of a rectangular wave, a sine curve and a triangular wave. The DC voltage of the vibration bias is a value between the background potential and image potential as mentioned above, and is preferably closer to the background potential than to the image potential to prevent the toner from adhering to the background.

When the vibration bias voltage has the waveform of a rectangular wave, a duty ratio is preferably not greater than 50 %. The duty ratio is a time ratio in which the toner is headed for the photoreceptor in one cycle of the vibration bias. A difference between the peak value and time average of the bias orienting the toner to the photoreceptor can be large, and therefore the toner moves more actively and faithfully adheres to the latent image to decrease a roughness and improve image resolution of the toner image. In addition, a difference between the peak value and time average of the bias orienting the carrier to the photoreceptor can be small, and therefore the carrier becomes inactive and probability of the carrier adherence to the background of the latent image can largely be decreased.

Fig. 3 is a schematic view illustrating an embodiment of the process cartridge of the present invention.

In Fig. 3, numeral (31) is a whole process cartridge, (32) is a photoreceptor, (33) is a charger, (34) is an image developer and (35) is a cleaner.

In the image forming apparatus having the process cartridge including the toner for developing an electrostatic latent image of the present invention, a photoreceptor rotates at a predetermined peripheral speed. A peripheral surface of the photoreceptor is positively or negatively charged by a charger uniformly while the photoreceptor is rotating to have a predetermined potential. Next, the photoreceptor receives an imagewise light from an irradiator such as a slit irradiator and a laser beam scanner to form an electrostatic latent image on the peripheral surface thereof. Then, the electrostatic latent image is developed by an image developer with a toner to form a toner image. Next, the toner image is transferred onto a transfer material fed between the photoreceptor and a transferer from a paper feeder in synchronization with the rotation of the photoreceptor. Then, the transfer material which received the toner image is separated from the surface of the photoreceptor and led to an image fixer fixing the toner image on the transfer material to form a copy image which is discharged out of the apparatus. The surface of the photoreceptor is cleaned by a cleaner to remove a residual toner after transfer, and is discharged to repeat forming images.

The fixer is a surf fixer rotating a fixing film as shown in Fig. 5. The fixing film is a heat resistant film having the shape of an endless belt, which is suspended and strained among a driving roller, a driven roller and a heater located therebetween underneath.

The driven roller is a tension roller as well, and the fixing film rotates clockwise according to a clockwise rotation of the driving roller in Fig. 5. The rotational speed of the fixing film is equivalent to that of a transfer material at a fixing nip area L where a pressure roller and the fixing film contact each other.

The pressure roller has a rubber elastic layer having good releasability such as silicone rubbers, and rotates counterclockwise while contacting the fixing nip area L at a total pressure of from 4 to 10 kg.

The fixing film preferably has a good heat resistance, releasability and durability, and has a total thickness not greater than 100 µm, and preferably not greater than 40 µm. Specific examples of the fixing film include films formed of a single-layered or a multi-layered film of heat resistant resins such as polyimide, polyetherimide, polyethersulphide (PES) and a tetrafluoroethyleneperfluoroalkylvinylether copolymer resin (PFA) having a thickness of 20 µm, on which (contacting an image) there is coated a release layer including a fluorocarbon resin such as a tetrafluoroethylene resin (PTFE) and a PFA and an electroconductive material and having a thickness of 10 µm or an elastic layer formed of a rubber such as a fluorocarbon rubber and a silicone rubber.

In Fig. 5, the heater is formed of a flat substrate and a fixing heater, and the flat substrate is formed of a material having a high heat conductivity and a high electric resistance such as alumina. The fixing heater formed of a resistance heater is located on a surface of the heater contacting the fixing film in the longitudinal direction of the heater. An electric resistant material such as Ag/Pd and Ta₂N is linearly or zonally coated on the fixing heater by a screen printing method, etc. Both ends of the fixing heater have electrodes (not shown) and the resistant heater generates heat when electricity passes though the electrodes. Further, a fixing temperature sensor formed of a thermistor is located on the other side of the substrate opposite to the side on which the fixing heater is located.

Temperature information of the substrate detected by the fixing temperature sensor is transmitted to a controller controlling an electric energy provided to the fixing heater to make the heater have a predetermined temperature.

Fig. 6 is a schematic view illustrating an embodiment of the image forming apparatus using a contact charger of the present invention. A photoreceptor to be charged and an image bearer rotates at a predetermined speed (process speed) in the direction of an arrow. A roller-shaped charging roller as a charger contacting the photoreceptor is basically formed of a metallic shaft and an electroconductive rubber layer circumferentially and concentrically overlying the metallic shaft. Both ends of the metallic shaft are rotatably supported by a bearing (not shown), etc. and the charging roller is pressed against the photoreceptor by a pressurizer (not shown) at a predetermined pressure. In Fig. 6, the charging roller rotates according to the rotation of the photoreceptor. The charging roller has a diameter of 16 mm because of being formed of a metallic shaft having a diameter of 9 mm and a middle-resistant rubber layer having a resistance of about 100, 000 Ω · cm coated on the metallic shaft.

The shaft of the charging roller and an electric source are electrically connected with each other, and the electric source applies a predetermined bias to the charging roller. Accordingly, a peripheral surface of the photoreceptor is uniformly charged to have a predetermined polarity and a potential.

The charger for use in the present invention may have any shapes besides the roller such as magnetic brushes and fur brushes, and is selectable according to a specification or a form of the electrophotographic image forming apparatus. The magnetic brush is formed of various ferrite particles such as Zn-Cu ferrite as a charging member, a non-magnetic electroconductive sleeve supporting the charging member and a magnet roll included by the non-magnetic electroconductive sleeve. The fur brush is a charger formed of a shaft subjected to an electroconductive treatment and a fur subjected to an electroconductive treatment with, e.g., carbon, copper sulfide, metals and metal oxides winding around or adhering to the shaft.

Fig. 7 is a schematic view illustrating another embodiment of the image forming apparatus using a contact charger of the present invention. A photoreceptor to be charged and an image bearer rotates at a predetermined speed (process speed) in the direction of an arrow. A brush roller formed of a fur brush contacts a photoreceptor at a predetermined pressure against an elasticity of the brush and a nip width.

The fur brush roller in this embodiment is a roll brush having an outer diameter of 14 mm and a longitudinal length of 250 mm, which is formed of a metallic shaft having a diameter of 6 mm and being an electrode as well, and a pile fabric tape of an electroconductive rayon fiber REC-B ® from Unitika Ltd. spirally winding around the shaft. The brush is 300 denier/50 filament and has a density of 155 fibers/mm². The roll brush is inserted into a pipe having an inner diameter of 12 mm while being rotated in a direction such that the brush and pipe are concentrically located, and is left in an environment of high humidity and high temperature to have inclined furs.

The fur brush roller has a resistance of 1 x 10⁵ Ω when an applied voltage is 100 V. The resistance is converted from a current when a voltage of 100 V is applied to the fur brush roller contacting a metallic drum having a diameter of 30 mm at a nip width of 3 mm.

The resistance needs to be not less than 10⁴ Ω and not greater than 10⁷ Ω to prevent defect images due to a insufficiently charged nip when a large amount of leak current flows into a defect such as a pin hole on the photoreceptor, and to sufficiently charge the photoreceptor.

Besides the REC-B ® from Unitika Ltd., specific examples of the brush material include REC-C ®, REC-M1 ® and REC-M10 ® therefrom; SA-7 ® from Toray Industries, Inc. ; Thunderon ® from Nihon Sanmo Dyeing Co., Ltd.; Belltron ® from Kanebo, Ltd.; Clacarbo ® from Kuraray Co., Ltd. ; carbon-dispersed rayon; and Roval ® from MITSUBISHI RAYON CO. , LTD. The brush preferably has a denier of from 3 to 10/fiber, a filament of from 10 to 100/batch and a density of from 80 to 600 fibers/mm. The fiber preferably has a length of from 1 to 10 mm.

The fur brush roller rotates in a counter direction of the rotation direction of the photoreceptor at a predetermined peripheral speed (surface speed) and contact the surface of the photoreceptor at a different speed. A predetermined charging voltage is applied to the fur brush roller from an electric source to uniformly charge the surface of the photoreceptor to have a predetermined polarity and a potential. In this embodiment, the fur brush roller contacts the photoreceptor to charge the photoreceptor, which is dominantly a direct injection charge, and the surface of the photoreceptor is charged to have a potential almost equal to an applied charging voltage to the fur brush roller.

The charger for use in the present invention may have any shapes besides the fur brush roller such as charging rollers and fur brushes, and is selectable according to a specification or a form of the electrophotographic image forming apparatus. The charging roller is typically formed of metallic shaft coated with a middle-resistant rubber layer having a resistance of about 100,000 Ω · cm. The magnetic brush is formed of various ferrite particles such as Zn-Cu ferrite as a charging member, a non-magnetic electroconductive sleeve supporting the ferrite particles and a magnet roll included by the non-magnetic electroconductive sleeve.

Fig. 8 is a schematic view illustrating another embodiment of the image forming apparatus using a contact charger of the present invention. A photoreceptor to be charged and an image bearer rotates at a predetermined speed (process speed) in the direction of an arrow. A brush roller formed of a magnetic brush contacts a photoreceptor at a predetermined pressure against an elasticity of the brush and a nip width.

The magnetic brush for use in the present invention as a contact charger includes magnetic particles coated with a middle-resistant resin including a mixture of Zn-Cu ferrite particles having an average particle diameter of 25 and 10 µm and a mixing weight ratio (25 µm/10 µm) of 1/0.05. The contact charger is formed of the coated magnetic particles, a non-magnetic electroconductive sleeve supporting the magnetic particles and a magnet roll included by the non-magnetic electroconductive sleeve. The coated magnetic particles are coated on the sleeve at a coated thickness of 1 mm to form a charging nip having a width of about 5 mm between the sleeve and photoreceptor, and a gap therebetween is about 500 µm. The magnet roll rotates in a counter direction of the rotation direction of the photoreceptor at a speed of twice as fast as a peripheral speed of a surface of the photoreceptor such that a surface of the sleeve frictionizes the surface of the photoreceptor and the magnetic brush uniformly contacts the photoreceptor.

The charger for use in the present invention may have any shapes besides the magnetic brush roller such as charging rollers and fur brushes, and is selectable according to a specification or a formof the electrophotographic image forming apparatus. The charging roller is typically formed of metallic shaft coated with a middle-resistant rubber layer having a resistance of about 100,000 Ω · cm. The fur brush is a charger formed of a shaft subjected to an electroconductive treatment and a fur subjected to an electroconductive treatment with, e.g., carbon, copper sulfide, metals and metal oxides winding around or adhering to the shaft.

Having generally described this invention, further understanding can be obtained by reference to certain specific examples which are provided herein for the purpose of illustration only and are not intended to be limiting. In the descriptions in the following examples, the numbers represent weight ratios in parts, unless otherwise specified.

### EXAMPLES

### Example 1

### Synthesis of toner binder resin

724 parts of an adduct of bisphenol A with 2 moles of ethyleneoxide, 276 parts isophthalic acid and 2 parts of dibutyltinoxide were mixed and reacted in a reactor vessel including a cooling pipe, a stirrer and a nitrogen inlet pipe for 8 hrs at a normal pressure and 230 °C. Further, after the mixture was depressurized by 10 to 15 mm Hg and reacted for 5 hrs, 32 parts of phthalic acid anhydride were added thereto and reacted for 2 hrs at 160 °C. Next, the mixture was reacted with 188 parts of isophoronediisocyanate in ethyl acetate for 2 hrs at 80°C to prepare a prepolymer including isocyanate (1). Next, 67 parts of the prepolymer (1) and 14 parts of isophoronediamine were mixed for 2 hrs at 50°C to prepare a urea-modified polyester resin (1) having a weight-average molecular weight of 64, 000. Similarly, 724 parts of an adduct of bisphenol A with 2 moles of ethyleneoxide and 276 parts of terephthalic acid were polycondensated for 8 hrs at a normal pressure and 230 °C, and further, after the mixture was depressurized by 10 to 15 mm Hg and reacted for 5 hrs to prepare a unmodified polyester resin (a) having a peak molecular weight of 5,000. 200 parts of the urea-modified polyester (1) and 800 parts of the unmodified polyester resin (a) were dissolved and mixed in 2,000 parts of a mixed solvent formed of ethyl acetate and MEK (1/1) to prepare a toner binder resin (1) ethyl acetate/MEK solution. The toner binder resin (1) ethyl acetate/MEK solution was partially depressurized and dried to isolate the toner binder resin (1). The toner binder resin (1) had a glass transition temperature (Tg) of 62 °C and an acid value of 10.

### Preparation for toner

240 parts of the toner binder resin (1) ethyl acetate/MEK solution, 20 parts of pentaelislitholtetrabehenate having a melting point of 81 °C and a melting viscosity of 25 cps and 10 parts of carbon black were mixed at 12,000 rpm in a beaker by a TK-type homomixer at 60°C to uniformly dissolve and disperse the mixture to prepare a toner material solution. 706 parts of ion-exchanged water, 294 parts of a slurry including 10 % hydroxyapatite Supertite 10 from Nippon Chemical Industrial Co., Ltd. and 0.2 parts of sodium dodecylbenzenesulfonate were uniformly dissolved in a beaker. Then, while the mixture was stirred at 12,000 rpm by a TK-type homomixer at 60 °C, the above-mentioned toner material solution was added thereto and the mixture was stirred for 10 min. Next, the mixture was moved into a flask with a stirrer and a thermometer, and heated at 98 °C to partially remove the solvent. Further, the mixture was stirred at 12, 000 rpm by a TK-type homomixer at a room temperature to completely remove the solvent. Then, the mixture was filtered, washed, dried and classified by a wind force to prepare a mother toner having a weight-average particle diameter (D4) of 6.35 µm, a number-average particle diameter (Dn) of 5.57 µm and D4/Dn of 1.14. Finally, 100 parts of the mother toner and 0.5 parts of hydrophobic silica were mixed by HENSCHEL mixer to prepare the toner of the present invention (1). The other detailed conditions and evaluations results are shown in Tables 1 to 3.

### Example 2

### Synthesis of toner binder resin

Similarly to Example 1, after 334 parts of an adduct of bisphenol A with 2 moles of ethyleneoxide, 334 parts of an adduct of bisphenol A with 2 moles of propyleneoxide, 274 parts isophthalic acid and 20 parts of trimellitic acid anhydride were polycondensated, 154 parts of isophoronediisocyanate were reacted with the polycondensated material to prepare a prepolymer (2). Next, 213 parts of the prepolymer (2), 9.5 parts of isophoronediamine and 0.5 parts dibutylamine were reacted similarly to Example 1 to prepare a urea-modified polyester resin (2) having a weigh-average molecular weight of 79,000. 200parts of the urea-modifiedpolyester (2) and 800 parts of the unmodified polyester resin (a) were dissolved and mixed in 2,000 parts of a mixed solvent formed of ethyl acetate and MEK (1/1) to prepare a toner binder resin (1) ethyl acetate/MEK solution. The toner binder resin (1) ethyl acetate/MEK solution was partially depressurized and dried to isolate the toner binder resin (2) . The toner binder resin (1) had a peak molecular weight of 5, 000, a glass transition temperature (Tg) of 62 °C and an acid value of 10.

### Preparation for toner

The procedure for preparation of the toner in Example 1 was repeated to prepare a mother toner (2) except for changing the toner binder resin (1) to the toner binder resin (2) and dissolution and dispersion temperature to 50 °C. Further, 1.0 parts of a zinc salt of a salicylic acid derivative was mixed and stirred in a heating atmosphere with 100 parts of the mother toner (2) as a charge controlling agent to fix the charge controlling agent thereon. The mother toner (2) had a weight-average particle diameter (D4) of 5.64 µm, a number-average particle diameter (Dn) of 4.98 µm and D4/Dn of 1.13. Finally, 100 parts of the mother toner and 1.0 parts of hydrophobic silica and 0.5 parts of a hydrophobic titanium oxide were mixed by HENSCHEL mixer to prepare the toner of the present invention (2). The other detailed conditions and evaluations results are shown in Tables 1 to 3.

### Example 3

### Synthesis of toner binder resin

30 parts of the urea-modified polyester resin (1) and 970 parts of the unmodified polyester resin (a) were dissolved and mixed in 2,000 parts of the mixed solvent formed of ethyl acetate andMEK (1/1) toprepareatonerbinderresin (3) ethyl acetate/MEK solution. The toner binder resin (3) ethyl acetate/MEK solution was partially depressurized and dried to isolate the toner binder resin (3) . The toner binder resin (1) had a peak molecular weight of 5,000, a glass transition temperature (Tg) of 62 °C and an acid value of 10.

### Preparation for toner

The procedure for preparation of the toner in Example 2 was repeated to prepare a toner (3) except for changing the toner binder resin (2) to the toner binder resin (3) and colorant to 8 parts of carbon black. The mother toner had a weight-average particle diameter (D4) of 6.72 µm, a number-average particle diameter (Dn) of 6.11 µm and D4/Dn of 1.10. The other detailed conditions and evaluations results are shown in Tables 1 to 3.

### Example 4

### Synthesis of toner binder resin

500 parts of the urea-modified polyester resin (1) and 500 parts of the unmodified polyester resin (a) were dissolved and mixed in 2, 000 parts of the mixed solvent formed of ethyl acetate and MEK (1/1) to prepare a toner binder resin (4) ethyl acetate/MEK solution. The toner binder resin (4) ethyl acetate/MEK solution was partially depressurized and dried to isolate the toner binder resin (4). The toner binder resin (4) had a peak molecular weight of 5,000, a glass transition temperature (Tg) of 62°C and an acid value of 10.

### Preparation for toner

The procedure for preparation of the toner in Example 1 was repeated to prepare a toner (4) except for changing the toner binder resin (1) to the toner binder resin (4) and colorant to 8 parts of carbon black. The mother toner had a weight-average particle diameter (D4) of 4.98 µm, a number-average particle diameter (Dn) of 4.35 µm and D4/Dn of 1.14. The other detailed conditions and evaluations results are shown in Tables 1 to 3.

### Example 5

### Synthesis of toner binder resin

750 parts of the urea-modified polyester resin (1) and 250 parts of the unmodified polyester resin (a) were dissolved and mixed in 2,000 parts of the mixed solvent formed of ethyl acetate and MEK (1/1) to prepare a toner binder resin (5) ethyl acetate/MEK solution. The toner binder resin (5) ethyl acetate/MEK solution was partially depressurized and dried to isolate the toner binder resin (5). The toner binder resin (5) had a peak molecular weight of 5,000, a glass transition temperature (Tg) of 62 °C and an acid value of 10.

### Preparation for toner

The procedure for preparation of the toner in Example 1 was repeated to prepare a toner (5) except for changing the toner binder resin (1) to the toner binder resin (5). The mother toner had a weight-average particle diameter (D4) of 5.93 µm, a number-average particle diameter (Dn) of 5.25 µm and D4/Dn of 1.14. The other detailed conditions and evaluations results are shown in Tables 1 to 3.

### Example 6

### Synthesis of toner binder resin

850 parts of the urea-modified polyester resin (1) and 150 parts of the unmodified polyester resin (a) were dissolved and mixed in 2,000 parts of the mixed solvent formed of ethyl acetate and MEK (1/1) to prepare a toner binder resin (6) ethyl acetate/MEK solution. The toner binder resin (6) ethyl acetate/MEK solution was partially depressurized and dried to isolate the toner binder resin (6). The toner binder resin (6) had a peak molecular weight of 5,000, a glass transition temperature (Tg) of 62 °C and an acid value of 10.

### Preparation for toner

The procedure for preparation of the toner in Example 1 was repeated to prepare a toner (6) except for changing the toner binder resin (1) to the toner binder resin (6). The mother toner had a weight-average particle diameter (D4) of 3.90 µm, a number-average particle diameter (Dn) of 3.38 µm and D4/Dn of 1.15. The other detailed conditions and evaluations results are shown in Tables 1 to 3.

### Example 7

### Synthesis of toner binder resin

724 parts of an adduct of bisphenol A with 2 moles of ethyleneoxide, 276 parts terephthalic acid were polycondensated for 2 hrs at a normal pressure and 230 °C. Further, the mixture was depressurized by 10 to 15 mm Hg and reacted for 5 hrs to prepare an unmodified polyester resin (b) having a peak molecular weight of 800. 200 parts of the urea-modified polyester resin (1) and 800 parts of the unmodified polyester resin (b) were dissolved and mixed in 2, 000 parts of the mixed solvent formed of ethyl acetate and MEK (1/1) to prepare a toner binder resin (7) ethylacetate/MEKsolution. The toner binder resin (7) ethyl acetate/MEK solution was partially depressurized and dried to isolate the toner binder resin (7). The toner binder resin (7) had a glass transition temperature (Tg) of 45 °C.

### Preparation for toner

The procedure for preparation of the toner in Example 1 was repeated to prepare a toner (7) except for changing the toner binder resin (1) to the toner binder resin (7). The mother toner had a weight-average particle diameter (D4) of 5.22 µm, a number-average particle diameter (Dn) of 4.50 µm and D4/Dn of 1.16. The other detailed conditions and evaluations results are shown in Tables 1 to 3.

### Example 8

210 parts of the toner binder solution prepared in Example 1 were diluted with 210 parts of ethyl acetate, and 210 parts of the diluted dispersion were emulsified and granulated similarly to Example 1. Then, the procedure for preparation of the toner in Example 1 was repeated to prepare a toner 8. The mother toner had a weight-average particle diameter (D4) of 4.25 µm, a number-average particle diameter (Dn) of 3.73 µm andD4/Dnof 1.14. The other detailed conditions and evaluations results are shown in Tables 1 to 3.

### Example 9

350 parts of the toner constituents after dispersed with the homomixer to remove the solvent therefrom in Example 1 were condensed to 175 parts with an evaporator, and 210 parts of the condensed dispersion were emulsified and granulated similarly to Example 1. Then, the procedure for preparation of the toner in Example 1 was repeated to prepare a toner 9. The mother toner had a weight-average particle diameter (D4) of 6.95 µm, a number-average particle diameter (Dn) of 5.65 µm and D4/Dn of 1.23. The other detailed conditions and evaluations results are shown in Tables 1 to 3.

### Example 10

210 parts of the toner constituents after dispersed with the homomixer to remove the solvent therefrom in Example 1 were diluted with 965 parts of ethyl acetate, and 210 parts of the diluted dispersion were emulsified and granulated similarly to Example 1. Then, the procedure for preparation of the toner in Example 1 was repeated to prepare a toner 10. The mother toner had a weight-average particle diameter (D4) of 3.95 µm, a number-average particle diameter (Dn) of 3.43 µm and D4/Dn of 1.15. The other detailed conditions and evaluations results are shown in Tables 1 to 3.

### Example 11

350 parts of the toner constituents after dispersed with the homomixer to remove the solvent therefrom in Example 1 were condensed to 125 parts with an evaporator, and 210 parts of the condensed dispersion were emulsified and granulated similarly to Example 1. Then, the procedure for preparation of the toner in Example 1 was repeated to prepare a toner 11. The mother toner had a weight-average particle diameter (D4) of 6.84 µm, a number-average particle diameter (Dn) of 5.61 µm and D4/Dn of 1.22. The other detailed conditions and evaluations results are shown in Tables 1 to 3.

### Comparative Example 1

### Synthesis of toner binder resin

354 parts of an adduct of bisphenol A with 2 moles of ethyleneoxide and 166 parts of isophthalic acid were polycondensated with 2 parts of dibutyltinoxide as a catalyst to prepare a comparative toner binder resin (1) having a peak molecular weight of 4,000. The comparative toner binder resin (1) had a glass transition temperature (Tg) of 57 °C.

### Preparation for toner

100 parts of the comparative toner binder resin (1) , 200 parts of ethyl acetate solution and 10 parts carbon black were mixed at 12,000 rpm in a beaker by a TK-type homomixer at 50 °C to uniformly dissolve and disperse the mixture. Then, the procedure for preparation of the toner in Example 1 was repeated to prepare a comparative toner (1). The mother toner had a weight-average particle diameter (D4) of 7.51 µm, a number-average particle diameter (Dn) of 6.05 µm and D4/Dn of 1.24. The other detailed conditions and evaluations results are shown in Tables 1 to 3.

### Comparative Example 2

343 parts of an adduct of bisphenol A with 2 moles of ethyleneoxide, 166 parts isophthalic acid and 2 parts of dibutyltinoxide were mixed and reacted in a reactor vessel including a cooling pipe, a stirrer and a nitrogen inlet pipe for 8 hrs at a normal pressure and 230 °C. Further, after the mixture was depressurized by 10 to 15 mm Hg and reacted for 5 hrs, the mixture was cooled to have 80 °C. Next, the mixture was reacted with 14 parts of toluenediisocyanate in toluene for 5 hrs at 150 °C, and then a solvent was removed therefrom to prepare a urethane-modified polyester resin having a weigh-average molecular weight of 98, 000. 363 parts of an adduct of bisphenol A with 2 moles of ethyleneoxide and 166 parts of isophthalic acid were polycondensated similarly to Example 1 to prepare a unmodified polyester resin having a peak molecular weight of 3,800 and an acid value of 7. 350 parts of the urethane-modified polyester and 650 parts of the unmodified polyester resin were dissolved and mixed in toluene, and a solvent was removed from the mixture to prepare a comparative toner binder resin (2). The toner binder resin (2) had a glass transition temperature (Tg) of 58 °C.

### Preparation for toner

100 parts of the comparative toner binder resin (2) and 8 parts of carbon black were preliminarily mixed by a HENSCHEL mixer and kneaded by a continuous kneader. Then, the kneaded mixture was pulverized by a jet pulverizer and classified by a wind classifier to prepare a mother toner. 100 parts of the mother toner and 1.0 parts of hydrophobic silica and 0.5 parts of a hydrophobic titanium oxide were mixed by HENSCHEL mixer to prepare a comparative toner (2). The mother toner had a weight-average particle diameter (D4) of 6.50 µm, a number-average particle diameter (Dn) of 5.50 µm and D4/Dn of 1.18. The other detailed conditions and evaluations results are shown in Tables 1 to 3.

### Comparative Example 3

### Synthesis of toner binder resin

354 parts of an adduct of bisphenol A with 2 moles of ethyleneoxide and 166 parts of terephthalic acid were polycondensated with 2 parts of dibutyltinoxide as a catalyst to prepare a comparative toner binder resin (3) having a peak molecular weight of 12,000. The comparative toner binder resin (3) had a glass transition temperature (Tg) of 62 °C and an acid value of 10.

### Preparation for toner

100 parts of the comparative toner binder resin (3), 200 parts of ethyl acetate solution and 4 parts of copper phthalocyanine pigment were mixed at 12, 000 rpm in a beaker by a TK-type homomixer at 50 °C to uniformly dissolve and disperse the mixture. Then, the procedure for preparation of the toner in Example 5 was repeated to prepare a comparative toner (3). The mother toner had a weight-average particle diameter (D4) of 6.12 µm, a number-average particle diameter (Dn) of 4.64 µm andD4/Dnof 1.32. The other detailed conditions and evaluations results are shown in Tables 1 to 3.

### Comparative Example 4

The procedure for preparation of the toner in Example 1 was repeated to prepare a comparative example toner (4) except for stirring at 18, 000 rpmwith the homomixer to completely remove the solvent. The other detailed conditions and evaluations results are shown in Tables 1 to 3.

### Comparative Example 5

The procedure for preparation of the toner in Example 1 was repeated to prepare a comparative example toner (5) except for mixing 0.2 parts of hydrophobic silica having a primary particle diameter of 35 µm with the HENSCHEL mixer with 100 parts of the mother toner. The other detailed conditions and evaluations results are shown in Tables 1 to 3.

### Comparative Example 6

The procedure for preparation of the toner in Example 1 was repeated to prepare a comparative example toner (6) except for mixing 0.2 parts of the hydrophobic silica with the HENSCHEL mixer with 100 parts of the mother toner. The other detailed conditions and evaluations results are shown in Tables 1 to 3.

### Comparative Example 7

The procedure for preparation of the toner in Example 1 was repeated to prepare a comparative example toner (7) except for mixing 5. 8 parts of the hydrophobic silica with the HENSCHEL mixer with 100 parts of the mother toner. The other detailed conditions-and evaluations results are shown in Tables 1 to 3.

The volume-average particle diameter (D4) and number-average particle diameter (Dn) of the toner were measured by a Coulter Counter TA-II connected with an interface producing a number distribution and a volume distribution from Nikkaki Bios Co., Ltd. and a personal computer PC9801 from NEC Corp. using a NaCl aqueous solution including a first class sodium by 1 % as an electrolyte as follows:
0.1 to 5 ml of a detergent, preferably alkylbenzene sulfonate was included as a dispersant in 100 to 150 ml of the electrolyte;
2 to 20 mg of a sample toner was included in the electrolyte and the toner was dispersed by an ultrasonic disperser for about 1 to 3 min to prepare a sample dispersion liquid;
the sample dispersion liquid was included in 100 to 200 ml of the electrolyte in another beaker so as to have a predetermined concentration;
a particle diameter distribution of the particles having a number-average particle diameter of from 2 to 40 µm was measured by the Coulter Counter TA-II using an aperture of 100 µm to determine volume and number distribution thereof; and
a weight-average particle diameter (D4) based on the volume distribution was determined.

A peripheral length of a circle having an area equivalent to that of a projected image optically detected is divided by an actual peripheral length of the toner particle to determine the circularity of the toner. -Specifically, the circularity of the toner is measured by a flow-type particle image analyzer FPIA-2000 from SYSMEX CORPORATION. A specific measuring method includes adding 0.1 to 0.5 ml of a surfactant, preferably an alkylbenzenesulfonic acid, as a dispersant in 100 to 150 ml of water from which impure solid materials are previously removed; adding 0.1 to 0.5 g of the toner in the mixture; dispersing the mixture including the toner with an ultrasonic disperser for 1 to 3 min to prepare a dispersion liquid having a concentration of from 3, 000 to 10, 000 pieces/µl; and measuring the toner shape and distribution with the above-mentioned measurer.

The SF-1 was be measured by randomly sampling toner images enlarged 1, 000 times as large as the original images, which have about 100 particles (or more) using scanning electron microscope S-800 from Hitachi, Ltd. ; and introducing the image information to an image analyzer Luzex III from NIRECO Corp. through an interface to analyze the information.

The image density and was measured by X-Rite 938, and the background density was also measured thereby to evaluate background fouling.

Whether toner filming over the surface of a developing roller occurred was visually observed.
- ○:: not occurred
- ×:: occurred

**Table 1**

| | Particle diameter | | | Shape | |
|---|---|---|---|---|---|
| | D4 | Dn | D4/Dn | Average circularity | SF-1 |
| Ex. 1 | 6.35 | 5.57 | 1.14 | 0.959 | 139 |
| Ex. 2 | 5.64 | 4.98 | 1.13 | 0.980 | 115 |
| Ex. 3 | 6.72 | 6.11 | 1.10 | 0.966 | 133 |
| Ex. 4 | 4.98 | 4.35 | 1.14 | 0.976 | 125 |
| Ex. 5 | 5.93 | 5.25 | 1.13 | 0.939 | 162 |
| Ex. 6 | 3.90 | 3.38 | 1.15 | 0.987 | 108 |
| Ex. 7 | 5.22 | 4.50 | 1.16 | 0.974 | 120 |
| Ex. 8 | 4.25 | 3.73 | 1.14 | 0.935 | 165 |
| Ex. 9 | 6.95 | 5.65 | 1.23 | 0.978 | 116 |
| Ex. 10 | 3.95 | 3.43 | 1.15 | 0.935 | 166 |
| Ex. 11 | 6.84 | 5.61 | 1.22 | 0.982 | 111 |
| Com. Ex. 1 | 7.51 | 6.05 | 1.24 | 0.955 | 144 |
| Com. Ex.2 | 6.50 | 5.50 | 1.18 | 0.924 | 173 |
| Com. Ex.3 | 6.12 | 4.64 | 1.32 | 0.960 | 128 |
| Com. Ex.4 | 5.66 | 4.67 | 1.21 | 0.932 | 165 |
| Com. Ex. 5 | 6.75 | 5.57 | 1.21 | 0.948 | 142 |
| Com. Ex.6 | 6.35 | 5.57 | 1.14 | 0.959 | 139 |
| Com. Ex.7 | 6.35 | 5.57 | 1.14 | 0.959 | 139 |

**Table 2**

| | External additive 1 | | | | External additive 2 | | | |
|---|---|---|---|---|---|---|---|---|
| | | Primary particle diameter (nm) | Secondary particle diameter (nm) | Content (parts by weight) | | Primary particle diameter (nm) | Secondary particle diameter (nm) | Content (parts by weight) |
| Ex. 1 | Hydrophobic silica | 10 | 120 | 0.5 | - | - | - | - |
| Ex. 2 | Hydrophobic silica | 10 | 120 | 1.0 | Titanium oxide | 15 | 150 | 0.5 |
| Ex. 3 | Hydrophobic silica | 10 | 120 | 1.5 | Titanium oxide | 15 | 150 | 0.5 |
| Ex. 4 | Hydrophobic silica | 15 | 80 | 2.0 | - | - | - | - |
| Ex. 5 | Hydrophobic silica | 15 | 80 | 2.5 | Titanium oxide | 15 | 150 | 0.5 |
| Ex. 6 | Hydrophobic silica | 15 | 80 | 5.0 | - | - | - | - |
| Ex. 7 | Titanium oxide | 15 | 150 | 1.0 | - | - | - | - |
| Ex. 8 | Hydrophobic silica | 10 | 150 | 0.5 | - | - | - | - |
| Ex. 9 | Hydrophobic silica | 10 | 150 | 0.5 | - | - | - | - |
| Ex.10 | Hydrophobic silica | 10 | 150 | 0.5 | - | - | - | - |
| Ex.11 | Hydrophobic silica | 10 | 150 | 0.5 | - | - | - | - |
| Com. Ex. 1 | Hydrophobic silica | 10 | 120 | 0.5 | - | - | - | - |
| Com . Ex. 2 | Hydrophobic silica | 10 | 120 | 1.0 | Titanium oxide | 15 | 150 | 0.5 |
| Com. Ex. 3 | Hydrophobic silica | 10 | 120 | 1.0 | Titanium oxide | 15 | 150 | 0.5 |
| Com. Ex. 4 | Hydrophobic silica | 10 | 120 | 0.5 | - | - | - | - |
| Com. Ex. 5 | Hydrophobic silica | 35 | - | 0.2 | - | - | - | - |
| Com. Ex. 6 | Hydrophobic silica | 10 | 120 | 0.2 | - | - | - | - |
| Com. Ex. 7 | Hydrophobic silica | 10 | 120 | 5.8 | - | - | - | - |

**Table 3**

| | Image density | | Background fouling | | Filming | Overall |
|---|---|---|---|---|---|---|
| | Initial | After 100,000 images were produced | Initial | After 100,000 images were produced | After 100,000 images were produced | |
| Ex. 1 | 1.44 | 1.36 | 0.02 | 0.05 | ○ | ○ |
| Ex. 2 | 1.37 | 1.38 | 0.01 | 0.00 | ○ | ○ |
| Ex. 3 | 1.45 | 1.41 | 0.00 | 0.01 | ○ | ○ |
| Ex. 4 | 1.45 | 1.43 | 0.01 | 0.01 | ○ | ○ |
| Ex. 5 | 1.42 | 1.46 | 0.00 | 0.01 | ○ | ○ |
| Ex. 6 | 1.48 | 1.46 | 0.01 | 0.00 | ○ | ○ |
| Ex. 7 | 1.46 | 1.45 | 0.00 | 0.00 | ○ | ○ |
| Ex. 8 | 1.42 | 1.38 | 0.02 | 0.05 | ○ | ○ |
| Ex. 9 | 1.43 | 1.38 | 0.02 | 0.02 | ○ | ○ |
| Ex. 10 | 1.41 | 1.36 | 0.01 | 0.04 | ○ | ○ |
| Ex. 11 | 1.43 | 1.37 | 0.01 | 0.02 | ○ | ○ |
| Com. Ex. 1 | 1.44 | 1.40 | 0.04 | 0.54 | ○ | × |
| Com. Ex. 2 | 1.36 | 1.31 | 0.02 | 0.16 | × | × |
| Com. Ex. 3 | 1.41 | 1.05 | 0.02 | 0.45 | × | × |
| Com. Ex. 4 | 1.31 | 1.01 | 0.03 | 0.55 | × | × |
| Com. Ex. 5 | 1.32 | 1.25 | 0.03 | 0.26 | × | × |
| Com. Ex. 6 | 1.09 | 0.82 | 0.04 | 0.05 | ○ | × |
| Com. Ex. 7 | 1.39 | 1.42 | 0.05 | 0.58 | × | × |

This document claims priority and contains subject matter related to Japanese Patent Applications Nos. 2003-349060 and 2003-400263, filed on October 8, 2003 and November 28, 2003, respectively.

## Claims

1. A toner comprising:
a particulate toner material having an average circularity of from 0.93 to 0.99, and including
a modified polyester binder resin (i), and
a colorant; and
an external additive in an amount of from 0.3 to 5.0 parts by weight per 100 parts by weight of the particulate toner material,
wherein the toner has a melting viscosity of from 70 to 140 Pa·s at 160°C,
a weight-average particle diameter (D4) of from 3 to 7 µm,
a ratio (D4/Dn) of the weight-average particle diameter to a number-average particle diameter (Dn) of the toner of from 1.01 to 1.25,
particles having a particle diameter not greater than 4 µm being present in an amount less than 10 % by number or particles having a particle diameter not less than 8 µm being present in an amount less than 2 % by volume.

2. The toner of Claim 1, wherein the toner has a shape factor (SF-1) of from 105 to 170.

3. The toner of Claim 1 or 2, wherein the modified polyester binder resin (i) is a modified polyester resin having a urea group.

4. The toner of any one of Claims 1 to 3, wherein the external additive is at least one of inorganic particulate material and a particulate polymer material.

5. The toner of any one of Claims 1 to 4, wherein the external additive is a hydrophobized silica.

6. The toner of any one of Claims 1 to 5, wherein the toner is prepared by a method comprising:
dissolving or dispersing toner constituents including a prepolymer in an organic solvent to prepare a solution or dispersion; and
dispersing the solution or dispersion in an aqueous medium to prepare the modified polyester binder resin (i).

7. The toner of any one of Claims 1 to 6, wherein the particulate toner material further includes an unmodified polyester binder resin (LL), and wherein a weight ratio (i/LL) of the modified polyester binder resin (i) to the unmodified polyester binder resin (LL) is from 5/95 to 80/20.

8. The toner of Claim 7, wherein the unmodified polyester binder resin (LL) has a peak molecular weight of from 1,000 to 20,000.

9. The toner of Claim 7 or 8, wherein the unmodified polyester binder resin (LL) has an acid value of from 10 to 30 mg KOH/g.

10. The toner of any one of Claims 7 to 9, wherein the unmodified polyester binder resin (LL) has a glass transition temperature (Tg) of from 35 to 55 °C.

11. The tonerof any one of Claims 1 to 10, further comprising a wax, wherein the wax is finely dispersed in the particulate toner material, and wherein a concentration of the wax at the surface of the particulate toner material is larger than a concentration thereof in the center of the particulate toner material.

12. The tonerof anyone of Claims 1 to 11, further comprising a charge controlling agent, wherein the charge controlling agent is fixed on the surface of the particulate toner material.

13. The toner of any one of claims 1 to 12, wherein the external additive has a primary particle diameter of from 5 to 20 nm and a secondary particle diameter of from 50 to 200 nm.

14. The toner of any one of Claims 1 to 13, wherein the toner is prepared by a volume contraction of from 10 to 90 % in an aqueous medium using a solid dispersant.

15. The toner of any one of Claims 1 to 14, wherein the toner is prepared by a method comprising:
dispersing a micro-droplet particulate material including at least an organic solvent, a binder resin and a colorant in an aqueous medium including a particulate resin; and
removing the organic solvent.

16. A container containing the toner according to any one of Claims 1 to 15.

17. A developer comprising the toner according to any one of Claims 1 to 15.

18. An image forming method comprising:
charging an electrophotographic photoreceptor to form an electrostatic latent image thereon;
developing the electrostatic latent image with the developer according to Claim 17 to form a toner image thereon;
transferring the toner image onto a transfer sheet; and
fixing the toner image on the transfer sheet.
cleaning the electrophotographic photoreceptor to remove the developer remaining thereon.

19. An image forming apparatus comprising:
a charger configured to charge an electrophotographic photoreceptor to form an electrostatic latent image thereon;
an image developer configured to develop the electrostatic latent image with the developer according to Claim 17 to form a toner image thereon;
a transferer configured to transfer the toner image onto a transfer sheet;
a fixer configured to fix the toner image on the transfer sheet; and
a cleaner configured to clean the electrophotographic photoreceptor to remove the developer remaining thereon.

20. The image forming apparatus of Claim 19, wherein the electrophotographic photoreceptor is an amorphous silicon photoreceptor.

21. The image forming apparatus of Claim 19 or 20, wherein the image developer applies an alternate current to the electrophotographic photoreceptor.

22. The image forming apparatus of any one of Claims 19 to 21, wherein the fixer comprises:
a heater;
a film contacting the heater; and
a pressurizer,
wherein the toner image is fixed on the transfer sheet between the film and the pressurizer upon application of heat.

23. The image forming apparatus of any one of Claims 19 to 22, wherein the charger charges the electrophotographic photoreceptor while contacting the electrophotographic photoreceptor.

24. A process cartridge detachably mountable in an image forming apparatus, comprising:
an image developer configured to develop an electrostatic latent image with the developer according to Claim 17; and
at least one of an electrophotographic photoreceptor, a charger and a cleaner.

## Patentansprüche

1. Toner, umfassend:
ein teilchenförmiges Tonermaterial mit einer mittleren Rundheit von 0,93 bis 0,99 und enthaltend
ein modifiziertes Polyester-Bindemittelharz (i) und
ein farbgebendes Mittel; und
ein externes Additiv in einer Menge von 0,3 bis 5,0 Gew.-Teilen pro 100 Gew.-Teilen des teilchenförmigen Tonermaterials,
wobei der Toner eine Schmelzviskosität von 70 bis 140 Pa·s bei 160°C,
ein Gewichtsmittel des Teilchendurchmessers (D4) von 3 bis 7 µm,
ein Verhältnis (D4/Dn) des Gewichtsmittels des Teilchendurchmessers zum Zahlenmittel des Teilchendurchmessers (Dn) des Toners von 1,01 bis 1,25 aufweist,
wobei Teilchen mit einem Teilchendurchmesser von nicht mehr als 4 µm in einer Menge von weniger als 10% bezogen auf die Zahl vorhanden sind oder Teilchen mit einem Teilchendurchmesser von nicht weniger als 8 µm in einer Menge von weniger als 2% bezogen auf das Volumen vorhanden sind.

2. Toner von Anspruch 1, wobei der Toner einen Formfaktor (SF-1) von 105 bis 170 aufweist.

3. Toner von Anspruch 1 oder 2, wobei das modifizierte Polyester-Bindemittelharz (i) ein modifiziertes Polyesterharz mit einer Harnstoffgruppe ist.

4. Toner von irgendeinem der Ansprüche 1 bis 3, wobei das externe Additiv mindestens eines von anorganischem teilchenförmigem Material und einem teilchenförmigen Polymermaterial ist.

5. Toner von irgendeinem der Ansprüche 1 bis 4, wobei das externe Additiv eine hydrophobisierte Kieselsäure ist.

6. Toner von irgendeinem der Ansprüche 1 bis 5, wobei der Toner hergestellt ist durch ein Verfahren umfassend:
das Lösen oder Dispergieren von Tonerbestandteilen einschließlich eines Präpolymers in einem organischen Lösungsmittel, um eine Lösung oder eine Dispersion zu bilden; und
das Dispergieren der Lösung oder Dispersion in einem wässrigen Medium, um das modifizierte Polyester-Bindemittelharz (i) herzustellen.

7. Toner von irgendeinem der Ansprüche 1 bis 6, wobei das teilchenförmige Tonermaterial ferner ein unmodifiziertes Polyester-Bindemittelharz (LL) beinhaltet und wobei das Gewichtsverhältnis (i/LL) des modifizierten Polyester-Bindemittelharzes (i) zum unmodifizierten Polyester-Bindemittelharz (LL) 5/95 bis 80/20 beträgt.

8. Toner von Anspruch 7, wobei das unmodifizierte Polyester-Bindemittelharz (LL) ein Peak-Molekulargewicht von 1.000 bis 20.000 aufweist.

9. Toner von Anspruch 7 oder 8, wobei das unmodifizierte Polyester-Bindemittelharz (LL) eine Säurezahl von 10 bis 30 mg KOH/g aufweist.

10. Toner von irgendeinem der Ansprüche 7 bis 9, wobei das unmodifizierte Polyester-Bindemittelharz (LL) eine Glasübergangstemperatur (Tg) von 35 bis 55°C aufweist.

11. Toner von irgendeinem der Ansprüche 1 bis 10, ferner umfassend ein Wachs,
wobei das Wachs fein in dem teilchenförmigen Tonermaterial verteilt ist und
wobei die Konzentration des Wachs an der Oberfläche des teilchenförmigen Tonermaterials größer ist als die Konzentration davon im Zentrum des teilchenförmigen Tonermaterials.

12. Toner von irgendeinem der Ansprüche 1 bis 11, ferner umfassend ein Ladungsregulierungsmittel, wobei das Ladungsregulierungsmittel auf der Oberfläche des teilchenförmigen Tonermaterials fixiert ist.

13. Toner von irgendeinem der Ansprüche 1 bis 12, wobei das externe Additiv einen primären Teilchendurchmesser von 5 bis 20 nm und einen sekundären Teilchendurchmesser von 50 bis 200 nm aufweist.

14. Toner von irgendeinem der Ansprüche 1 bis 13, wobei der Toner durch eine Volumenkontraktion von 10 bis 90% in einem wässrigen Medium unter Verwendung eines festen Dispergiermittels hergestellt ist.

15. Toner von irgendeinem der Ansprüche 1 bis 14, wobei der Toner hergestellt ist durch ein Verfahren umfassend:
das Dispergieren von Mikrotröpfchen von teilchenförmigem Material enthaltend mindestens ein organisches Lösungsmittel, ein Bindemittelharz und ein farbgebendes Mittel in einem wässrigen Medium enthaltend ein teilchenförmiges Harz; und
Entfernen des organischen Lösungsmittels.

16. Behälter, enthaltend den Toner nach irgendeinem der Ansprüche 1 bis 15.

17. Entwickler, umfassend den Toner nach irgendeinem der Ansprüche 1 bis 15.

18. Bildaufzeichnungsverfahren, umfassend:
das Aufladen eines elektrophotographischen Photorezeptors für die Bildung eines elektrostatischen latenten Bildes darauf;
das Entwickeln des elektrostatischen latenten Bildes mit dem Entwickler nach Anspruch 17, um ein Tonerbild darauf zu erzeugen;
das Übertragen des Tonerbildes auf einen Übertragungsbogen; und
das Fixieren des Tonerbildes auf dem Übertragungsbogen;
das Reinigen des elektrophotographischen Photorezeptors, um darauf verbleibenden Entwickler zu entfernen.

19. Bildaufzeichnungsvorrichtung, umfassend:
eine Aufladevorrichtung, die konfiguriert ist einen elektrophotographischen Photorezeptor aufzuladen, um darauf ein elektrostatisches latentes Bild zu bilden;
eine Bildentwicklungsvorrichtung, die konfiguriert ist das elektrostatische latente Bild mit dem Entwickler nach Anspruch 17 zu entwickeln, um ein Tonerbild darauf zu bilden;
eine Übertragungsvorrichtung, die konfiguriert ist das Tonerbild auf einen Übertragungsbogen zu übertragen;
eine Fixiervorrichtung, die konfiguriert ist das Tonerbild auf dem Übertragungsbogen zu fixieren; und
eine Reinigungsvorrichtung, die konfiguriert ist den elektrophotographischen Photorezeptor zu reinigen, um den darauf verbleibenden Entwickler zu entfernen.

20. Bildaufzeichnungsvorrichtung von Anspruch 19, wobei der elektrophotographische Photorezeptor ein Photorezeptor aus amorphem Silicium ist.

21. Bildaufzeichnungsvorrichtung von Anspruch 19 oder 20, wobei die Bildentwicklungsvorrichtung an den elektrophotographischen Photorezeptor einen Wechselstrom anlegt.

22. Bildaufzeichnungsvorrichtung von irgendeinem der Ansprüche 19 bis 21,
wobei die Fixiervorrichtung umfasst:
eine Heizvorrichtung;
eine Folie, die die Heizvorrichtung kontaktiert; und
eine Druckanwendungsvorrichtung,
wobei das Tonerbild auf dem Übertragungsbogen zwischen der Folie und der Druckanwendungsvorrichtung unter Erwärmung fixiert wird.

23. Bildaufzeichnungsvorrichtung von irgendeinem der Ansprüche 19 bis 22,
wobei die Aufladevorrichtung den elektrophotographischen Photorezeptor auflädt, während der elektrophotographische Photorezeptor kontaktiert wird.

24. Prozesskartusche, die ablösbar in einer Bildaufzeichnungsvorrichtung montiert werden kann, umfassend:
eine Bildentwicklungsvorrichtung, die konfiguriert ist ein elektrostatisches latentes Bild mit dem Entwickler nach Anspruch 17 zu entwickeln; und
mindestens eines von einem elektrophotographischen Photorezeptor, einer Aufladevorrichtung und einer Reinigungsvorrichtung.

## Revendications

1. Toner comprenant :
un matériau de toner particulaire ayant une circularité moyenne de 0,93 à 0,99, et comportant :
une résine de liant polyester modifiée (i), et
un colorant ; et
un additif externe en une quantité de 0,3 à 5,0 parties en poids pour 100 parties en poids du matériau de toner particulaire,
dans lequel le toner a une viscosité de fusion de 70 à 140 Pa·s à une température de 160°C,
un diamètre moyen des particules en poids (D4) de 3 à 7 µm,
un rapport (D4/Dn) du diamètre moyen des particules en poids sur un diamètre moyen des particules en nombre (Dn) du toner de 1,01 à 1,25,
des particules ayant un diamètre des particules n'excédant pas 4 µm qui sont présentes en une quantité inférieure à 10 % en nombre ou des particules ayant un diamètre des particules qui n'est pas inférieur à 8 µm qui sont présentes en une quantité inférieure à 2 % en volume.

2. Toner selon la revendication 1, dans lequel le toner a un facteur de forme (SF-1) de 105 à 170.

3. Toner selon la revendication 1 ou 2, dans lequel la résine de liant polyester modifiée (i) est une résine polyester modifiée ayant un groupe urée.

4. Toner selon l'une quelconque des revendications 1 à 3, dans lequel l'additif externe est au moins un parmi un matériau particulaire inorganique et un matériau polymère particulaire.

5. Toner selon l'une quelconque des revendications 1 à 4, dans lequel l'additif externe est une silice rendue hydrophobe.

6. Toner selon l'une quelconque des revendications 1 à 5, dans lequel le toner est préparé grâce à un procédé comprenant les étapes consistant à :
dissoudre ou disperser des constituants de toner comportant un pré-polymère dans un solvant organique afin de préparer une solution ou une dispersion ; et
disperser la solution ou la dispersion dans un milieu aqueux afin de préparer la résine de liant polyester modifiée (i).

7. Toner selon l'une quelconque des revendications 1 à 6, dans lequel le matériau de toner particulaire comporte en outre une résine de liant polyester non modifiée (LL), et dans lequel un rapport en poids (i/LL) de la résine de liant polyester modifiée (i) sur la résine de liant polyester non modifiée (LL) est de 5/95 à 80/20.

8. Toner selon la revendication 7, dans lequel la résine de liant polyester non modifiée (LL) a un poids moléculaire maximum de 1 000 à 20 000.

9. Toner selon la revendication 7 ou 8, dans lequel la résine de liant polyester non modifiée (LL) a un indice d'acide de 10 à 30 mg KOH/g.

10. Toner selon l'une quelconque des revendications 7 à 9, dans lequel la résine de liant polyester non modifiée (LL) a une température de transition vitreuse (Tg) de 35 à 55°C.

11. Toner selon l'une quelconque des revendications 1 à 10, comprenant en outre une cire, dans lequel la cire est soigneusement dispersée dans le matériau de toner particulaire, et dans lequel une concentration en cire au niveau de la surface du matériau de toner particulaire est supérieure à une concentration de celle-ci au centre du matériau de toner particulaire.

12. Toner selon l'une quelconque des revendications 1 à 11, comprenant en outre un agent contrôleur de charge dans lequel l'agent contrôleur de charge est fixé à la surface du matériau de toner particulaire.

13. Toner selon l'une quelconque des revendications 1 à 12, dans lequel l'additif externe a un diamètre des particules primaires de 5 à 20 nm et un diamètre des particules secondaires de 50 à 200 nm.

14. Toner selon l'une quelconque des revendications 1 à 13, dans lequel le toner est préparé grâce à une contraction de volume de 10 à 90 % dans un milieu aqueux en utilisant un agent dispersant solide.

15. Toner selon l'une quelconque des revendications 1 à 14, dans lequel le toner est préparé grâce à un procédé comprenant les étapes consistant à :
disperser un matériau particulaire en micro-gouttelettes comportant au moins un solvant organique, une résine de liant et un colorant dans un milieu aqueux comportant une résine particulaire ; et
retirer le solvant organique.

16. Récipient contenant le toner selon l'une quelconque des revendications 1 à 15.

17. Révélateur comprenant le toner selon l'une quelconque des revendications 1 à 15.

18. Procédé de formation d'images comprenant les étapes consistant à :
charger un photorécepteur électrophotographique afin d'y former une image latente électrostatique ;
révéler l'image latente électrostatique à l'aide du révélateur selon la revendication 17 pour y former une image toner ;
transférer l'image toner sur une feuille de transfert ; et
fixer l'image toner sur la feuille de transfert ;
nettoyer le photorécepteur électrophotographique pour en retirer le reste de révélateur.

19. Appareil de formation d'images comprenant :
un chargeur configuré afin de charger un photorécepteur électrophotographique afin d'y former une image latente électrostatique ;
un révélateur d'image configuré afin de révéler l'image latente électrostatique à l'aide du révélateur selon la revendication 17 afin d'y former une image toner ;
un dispositif de transfert configuré afin de transférer l'image toner sur une feuille de transfert ;
un dispositif de fixage configuré afin de fixer l'image toner sur la feuille de transfert ; et
un dispositif de nettoyage configuré afin de nettoyer le photorécepteur électrophotographique pour en retirer le reste de révélateur.

20. Appareil de formation d'images selon la revendication 19, dans lequel le photorécepteur électrophotographique est un photorécepteur au silicium amorphe.

21. Appareil de formation d'images selon la revendication 19 ou 20, dans lequel le révélateur d'image applique un courant alternatif au photorécepteur électrophotographique.

22. Appareil de formation d'images selon l'une quelconque des revendications 19 à 21, dans lequel le dispositif de fixage comprend :
un élément chauffant ;
un film entrant en contact avec l'élément chauffant ; et
un générateur de pression,
dans lequel l'image toner est fixée sur la feuille de transfert entre le film et le générateur de pression lors d'une application de chaleur.

23. Appareil de formation d'images selon l'une quelconque des revendications 19 à 22, dans lequel le chargeur charge le photorécepteur électrophotographique tout en entrant en contact avec le photorécepteur électrophotographique.

24. Cartouche de traitement pouvant être montée de manière détachable dans un appareil de formation d'images, comprenant :
un révélateur d'image configuré afin de révéler une image latente électrostatique à l'aide du révélateur selon la revendication 17 ; et
au moins un parmi un photorécepteur électrophotographique, un chargeur et un dispositif de nettoyage.
